



US006211894B1

(12) **United States Patent**  
Yamaya et al.

(10) **Patent No.:** US 6,211,894 B1  
(45) **Date of Patent:** Apr. 3, 2001

(54) **IMAGE FORMING METHOD**

(75) Inventors: **Yoshihiro Yamaya; Shigeru Mano; Kaori Fukumuro; Hiroshi Watanabe**, all of Hino (JP)

(73) Assignee: **Konica Corporation (JP)**

(\*) Notice: Subject to any disclaimer, the term of this patent is extended or adjusted under 35 U.S.C. 154(b) by 0 days.

(21) Appl. No.: **09/243,368**

(22) Filed: **Feb. 1, 1999**

(30) **Foreign Application Priority Data**

Feb. 1, 1998 (JP) ..... 10-034096  
Dec. 31, 1998 (JP) ..... 10-377516

(51) **Int. Cl. 7** ..... **B41J 2/32**

(52) **U.S. Cl.** ..... **347/193; 347/191**

(58) **Field of Search** ..... **347/175, 176, 347/172, 191, 193, 213, 221, 188**

(56) **References Cited**

## U.S. PATENT DOCUMENTS

5,634,731 \* 6/1997 Kita et al. ..... 347/213

## FOREIGN PATENT DOCUMENTS

6-155778 \* 6/1994 (JP) ..... 347/213

\* cited by examiner

Primary Examiner—N. Le

Assistant Examiner—Anh T. N. Vo

(74) Attorney, Agent, or Firm—Jordan B. Bierman; Bierman, Muserlian and Lucas, LLP

(57) **ABSTRACT**

In an image forming method in that an image-receiving layer of an image-receiving element is in contact with an ink sheet comprising a thermally transferable dye, and the dye is transferred to the image-receiving layer in accordance with imagewise-heating by a thermal head, the image-receiving layer having dye image formed by dye transfer is subjected to re-heating through a thin film material by thermal head.

**7 Claims, 2 Drawing Sheets**



FIG. 1 (a)



FIG. 1 (b)



FIG. 1 (c)



FIG. 2 (a)



FIG. 2 (b)



FIG. 2 (c)



## IMAGE FORMING METHOD

## FIELD OF THE INVENTION

The present invention relates to an image forming method in which an image is formed by employing thermal transfer, and more specifically to a technology for the improvement in the keeping quality of a transferred image without deteriorating the surface characteristics of the image receiving sheet.

## BACKGROUND OF THE INVENTION

As a multicolor or single-color image forming technology, this technology has been known in that an ink sheet containing a sublimable dye is in contact with an image-receiving layer of a image-receiving element and is heated by a thermal head, etc. so that the sublimable dye is transferred imagewise to the image-receiving layer.

In such the transferred image forming technology, the sublimable dye employed in the ink sheet plays an important roles, and image preservation quality is not sufficient from the conventional sublimable dye. As for improving this problem it is disclosed in Japanese Patent Publication Open to Public Inspection Nos. 59-78893, 59-109394, 60-2398 etc. that a metal chelate is formed by allowing a metal ion-containing compound (metal source) to react with a thermally transferable dye which is capable of chelate reaction (post chelate dye) to form a dye image.

It has been known that the image preservation quality of the post chelate sublimable dye image is improved as a chelation ratio becomes higher which is obtained by allowing a post chelate dye supplied from the ink sheet to react with the metal source in the image-receiving layer.

As a method to increase the chelation ratio, a technology has been proposed in that an image formed by transfer is treated at high temperature employing a thermostat or another heating device (Japanese Patent Publication Open to Public Inspection No. 4-89292 and Japanese Patent Application No. 5-258397). However, in this method, there is a disadvantage since another device is required in addition to a thermal transfer printer and further two steps-working is required for forming image with inferior handling. In this method, cost becomes higher since a sheet form protective material is necessary attaching between the image receiving sheet and roller and press plate to avoid contamination of the roller and press plate by dye transfer in the heating procedure.

A method heating the image formed by thermal transfer recording, a method employing thermal head is proposed. For example, it is disclosed in Japanese Patent Publication 4-55870, employing a sublimation transfer paper having dye areas of each color and an area having no coating, a transferred image receiving sheet is heated again through the non-coated area by means of a thermal head after the dye transfer. This method is advantageous because the re-heating is carried out within a same apparatus as the thermal transfer recording apparatus.

In case that the re-heating is carried out employing a thermal head with the same applied energy as that is applied when dye transferring with the maximum density, the image receiving layer or support is deteriorate so that an original surface characteristics of the image receiving sheet is lost, uneven band image appears at the high density area or sticking occurred at worst due to reducing the slippability between the image receiving layer and ink layer or back side of ink sheet and thermal head, because an excess energy all

energy for dye transfer is used for the re-heating. For this reason the applied energy is set at lower condition than that gives maximum density of dye transfer. When the applied energy is reduced to avoid the phenomenon mentioned above, chelation of the post chelate dye is not performed sufficiently and the preservation quality of the obtained image becomes reduced.

## SUMMARY OF THE INVENTION

An object of the present invention is to provide a technology to dissolve such problem mentioned above, and to improve the preservation quality of a thermally transferred image formed on an image-receiving layer without reducing the original surface characteristics of image receiving sheet as itself, fusion of the image receiving layer with ink layer, sticking between back side of ink layer and thermal head or occurrence of uneven image.

The invention and its embodiment are described.

An ink sheet used in the present invention comprises an ink layer containing a thermal transfer dye provided on a support. An image-receiving element comprises, provided on a support, an image-receiving layer which accepts the thermal transfer dye.

The image forming process comprises the following steps;

An image-receiving layer of an image-receiving element having the image-receiving layer and an ink layer of the ink sheet are brought into contact and are subjected to imagewise-heating by a thermal head and the dye of the ink sheet is transferred to the image-receiving layer to form an image on the image-receiving layer,

the image receiving element in which a transferred image was formed is subjected re-heating by a thermal head through a thin film material which is brought into contact to an image forming surface of the image receiving sheet,

wherein pulse supplying period per one line of the thermal head of re-heating is shorter than that of the thermal head of imagewise heating, and supplying energy to the thermal head of re-heating is lower than that of the thermal head of imagewise heating which gives maximum density.

The pulse supplying period per one line of the thermal head of re-heating is preferably 65 to 95% of that of the thermal head of imagewise heating.

The supplying energy to the thermal head of re-heating is preferably 40 to 80% of that of the thermal head of imagewise heating which gives maximum density.

In one of the preferable embodiment the ink layer contains a thermally transfer dye precursor, and the image receiving layer contains a dye fixing compound capable of forming a dye by reacting with the dye thermally transfer dye precursor.

The preferable example of the thermally transfer dye precursor is a thermally transfer dye capable of chelation. The preferable example of the dye fixing compound is a metal ion containing compound capable of chelating with the thermally transfer dye capable of chelation.

In one of the preferable embodiment the ink layer contains a dye capable of chelating as the thermal transfer dye. The image receiving layer preferably contains a metal ion containing compound which reacts with the dye capable of chelating.

The thin film material preferably comprises a layer containing a metal ion containing compound.

In one of the embodiment of the invention, the thin film material is provided in a part of the ink layer. In this case,

the ink sheet comprises dye-containing region and the thin film material region. The dye-containing region is composed of, for example, an yellow dye-containing region, a magenta dye-containing region and a cyan dye-containing region, and the thin film material region is formed next those dye-containing regions.

The thin film material preferably comprises a releasing agent.

#### BRIEF EXPLANATION OF THE DRAWINGS

FIGS. 1(a), 1(b) and 1(c) each is example of the arrangement of ink sheet and thin film material employed in the invention.

FIGS. 2(a), 2(b) and 2(c) each is a schematic diagram of one example of a heat transfer recording apparatus employed in the invention.

#### DETAILED DESCRIPTION OF THE INVENTION

The present invention is described in detail below.

The re-heating process is carried out employing a thermal head through a thin film material after dye transfer. The thermal head may be the same one that employed for dye transfer process or another thermal head may be provided for the re-heating than that employed for dye transfer process.

In control of the thermal head, pulse supplying period per one line of the thermal head of re-heating is shorter than that of the thermal head of imagewise heating (preferably 65 to 95%), and applying energy to the thermal head of re-heating is lower than that of the thermal head of imagewise heating which gives maximum density (preferably 40 to 80%). According to this control method the problem mentioned above can be dissolved without reducing the preserve ability of the image after re-heating. When multiple dye image are transferred in the different pulse supplying period in color, the ratio is calculated by the pulse supplying period of the slowest pulse supplying period for dye transfer for the comparison. The comparison of supplying energy is taken with the highest energy for dye transfer.

The purpose of control the applying energy is to shorten pulse power supplying time per 1 dot, i.e., pulse width, whereby applied energy is reduced, and to shorten the pulse supplying period. In case that the pulse power supplying time is shortened but the pulse supplying period is not shortened, heat discharging time of the head becomes long, and consequently heating is not uniform but uneven. In case that the pulse supplying period is shortened but the pulse power supplying time is not shortened, heat is accumulated within the head, uneven heating or overload of the head may occur.

The control method in which feeding speed is increased (i.e., pulse supplying period is reduced) and applying energy is reduced seems counteraction for the purpose of increasing chelate ratio. However, applying energy should be image-wise controlled in heating at dye transfer process, therefore energy applying time should be taken for certain period to avoid affecting neighboring dots. In the re-heating process heating should be carried out for whole image area uniformly, and therefore, the applying time is not necessary so long as that of dye transfer process, to the contrary taking shorter time, even though the energy is reduced, next energy is applied within the time period in which the energy applied is not diffused, a higher energy is applied to the image receiving sheet as a whole than the case that higher energy is applied for shorter time.

The thin film material includes the material having micro-void layer such as synthesis paper made of polyolefin or polystyrene, and further those conventionally employed for an ink sheet employing a sublimation dye. Preferable examples of the thin film material includes thin paper such as condenser paper, glassine paper and paraffin paper, a drafted or undrafted film of plastics including polyester having high resistance to heat such as polyethyleneterphthalate, polyethylenenaphthalate, polybutyleneterephthalate, polyphenylenesulfide, polyetherketone and polyethersulfone, polypropylene, polycarbonate, celluloseacetate, polyethylene derivative, polyvinylchloride, polyvinilidenechloride, polystyrene, polyamide, polyimide, polymethylpentene, ionomer, or laminated film of these material.

The thickness of the thin film material is optionally selected to obtain an adequate strength, thermal conductivity, heat resistance etc., according to the material. Usually 1 to 100  $\mu\text{m}$  is preferably employed.

The thin film material may be supplied in each sheet leaf by leaf or in roll. When the same thermal head as that employed for dye transfer process is employed for re-heating process, the thin film material is supplied in order of dye and the thin film material. In this case, the thin film material is prepared from the same material as the support of the ink sheet because of convenience of preparation.

Practical example that the thin film material is supplied in order of dye and the thin film material will be illustrated in accordance with the Drawing. FIGS. 1(a), 1(b) and 1(c) are examples of the ink sheet employed in the invention. In FIG. 1(a) the ink sheet in which each of yellow (2Y), magenta (2M) and cyan (2C) ink area having corresponding dye layer are arranged in order, and an area for re-heating process having same size of each ink layer is provided between a cyan dye layer and a yellow dye layer. The area for re-heating is called re-heating layer in this specification. While there is no space between each ink area or re-heating area in the ink sheet illustrated in FIG. 1(a), appropriate space may be provided in accordance with the control system of the thermal transfer recording apparatus. It is preferable to provide a control mark for the purpose of precise control of detecting a initial position in the ink sheet. While the ink areas and re-heating area are provided on a same support in FIGS. 1(a) and 1(b), the ink areas 2 and re-heating area 1 may be provided on separate supports as illustrated in FIG. 1(c).

As a thermal transfer recording apparatus, for example, the apparatus shown in FIG. 2 can be employed. In FIGS. 2(a) to 2(c), the reference numeral 10 is an ink sheet supply roll, 15 is an ink sheet, 11 is a winding roll which winds a used ink sheet 15, 12 is a thermal head, 13 is a platen roller and 14 is an image-receiving element inserted between the thermal head 12 and the platen roller 13.

While employing the thermal transfer apparatus shown in FIG. 2(a), for forming a transfer image employing, for example, the ink sheet shown in FIG. 1(a) as an ink sheet, at first, an yellow dye-containing region 2Y of the ink sheet and the image-receiving layer of the image-receiving element are brought into contact and they are heated by the thermal head in accordance with image data and the yellow dye in the ink layer of the aforesaid region is transferred to the image-receiving element to form the yellow image; thereafter, in the same way, the magenta dye is transferred imagewise from the ink layer of the magenta dye-containing region 2M to the yellow image; thereafter, in the same way, the cyan dye is transferred imagewise from the ink layer of

the cyan dye-containing region 2C to the resulting image; lastly, the formation of the transfer image is completed by re-heating whole area of the resulting image through re-heating layer 1 by means of the thermal head.

While employing the thermal transfer apparatus shown in FIG. 2(a), for forming a transfer image employing, for example, the ink sheet shown in FIG. 1(b) as an ink sheet, at first, an yellow dye-containing region 2Y of the ink sheet and the image-receiving layer of the image-receiving element are brought into contact and they are heated by the thermal head in accordance with image data and the yellow in the ink layer of the aforesaid region is transferred to the image-receiving sheet to form the yellow image, the whole area of the transfer image is subjected by re-heating through re-heating layer 1 by means of re-heating apparatus; thereafter, in the same way, the magenta dye is transferred imagewise from the ink layer of the magenta dye-containing region 2M to the yellow image and the whole area of the image is subjected by re-heating; thereafter, in the same way, the cyan dye is transferred imagewise from the ink layer of the cyan dye-containing region 2C to the resulting image; lastly, the formation of the transfer image is completed by re-heating whole area of the resulting image through re-heating layer 1 by means of re-heating apparatus.

FIG. 2(b) illustrates the case employing ink sheet shown in FIG. 1(c). At first, an yellow dye-containing region 2Y of the ink sheet and the image-receiving layer of the image-receiving element are brought into contact and they are heated by the thermal head in accordance with image data and the yellow dye in the ink layer is transferred to the image-receiving element to form the yellow image; thereafter, in the same way, the magenta dye is transferred imagewise from the ink layer of the magenta dye-containing region 2M to the yellow image; thereafter, in the same way, the cyan dye is transferred imagewise from the ink layer of the cyan dye-containing region 2C to the resulting image; lastly, the formation of the image is completed by re-heating whole area of the resulting image through re-heating layer 1 employing re-heating apparatus.

FIG. 2(c) represents the case that the record is performed using ink sheet having dye of individual color and each apparatus corresponding to the individual colored ink sheet. In this case, yellow dye image is formed by transferring the dye in the ink sheet according to the image data by the transfer apparatus for yellow dye, in the same way magenta dye in the magenta ink sheet is transferred imagewise on the yellow image by the transfer apparatus for magenta dye, next cyan dye in the cyan ink sheet is transferred imagewise on the formed image by the transfer apparatus for cyan dye, and finally the formation of the image is completed by re-heating whole area of the resulting image through re-heating layer 1 employing re-heating apparatus in the same way as in the case of FIG. 2(b).

The releasing layer containing a releasing agent is preferably provided on the thin layer material so as to avoid the fusion of the thin layer material with the image-receiving layer during the re-heating process. As this kind of the releasing agent, there are illustrated silicone oil (including those termed silicone resins); solid wax such as polyethylene wax, polypropylene wax, amide wax, Teflon powder, etc.; silicate compounds or those composite compounds; fluorine series or phosphoric acid ester series surface active agents; coupling agents; long chain alkyl compounds; polyoxyalkyl polyols, etc., and of these, the silicone oil is preferred.

The silicone oil is classified into a simply added type (simple addition type) and a hardening or reacting type

(hardening-reaction type). In the case of the simple addition type, a modified silicone oil is preferably employed, are illustrated polyester-modified silicone resins (or silicone-modified polyester resins), acryl-modified silicone resins (or silicone-modified acrylic resins), urethane-modified silicone resins (or silicone-modified urethane resins), cellulose-modified silicone resin (or silicone-modified cellulose resins), alkyd-modified silicone resins (or silicone-modified alkyd resins), epoxy-modified silicone resins (or silicone-modified epoxy resins), etc.

As the hardening-reaction type silicone oil, for examples are illustrated modified silicone oil having a reactive group mentioned below.

(a) amino-modified silicone having an amino group



(b) epoxy-modified silicone having an epoxy group



(c) modified silicone having another reactive group

Modified silicone represented by the following general formula and determined by a reaction group: R<sub>6</sub>.



R<sub>6</sub>: isocyano-modified silicone of —NCO

R<sub>6</sub>: alcohol-modified silicone of —OH

R<sub>6</sub>: carboxyl-modified silicone of —COOH

Further, in the general formulas (structural formulas) of the above-mentioned (a) to (c), R<sub>1</sub> to R<sub>5</sub> each independently represents an organic group which is mainly a methyl group or an alkyl group other than the methyl group or a phenyl group and 1, m and n each independently represents an integer of 1 or more determined appropriately according to the molecular weight of a releasing resin. Further, the atom group of 1 and m parts is randomly copolymerized.

The silicone mentioned above is employed in suitable combination for carrying out the hardening reaction according to a reaction scheme. As the reaction scheme, the modified silicone having an amino group or a hydroxyl group reacts with each of the modified silicone having an epoxy group, an isocyanato group or a carboxyl group. <sup>5</sup>

As those of the catalyst hardening type, the following two types (d) and (e) of silicones are illustrated.

(d) those are alcohol-modified silicones which can <sup>10</sup> undergo dehydration polymerization reaction between two silicones.



(catalysts: carboxylic acid salts, etc. of titanate, zinc, <sup>20</sup> iron, etc.)

(e) those are composed of vinyl-modified silicone and vinyl-modified silicone in which a part of the organic group is —H. <sup>25</sup>



(catalysts: metal catalysts of platinum series, etc.)

Further, in the above-mentioned general formulas <sup>35</sup> (structural formulas) (d) to (e), R<sub>1</sub> to R<sub>6</sub> each independently represents an organic group which is mainly a methyl group and may be an alkyl group or a phenyl group other than the methyl group. However, in (e), in the case of the vinyl-modified silicone, any of R<sub>1</sub> to R<sub>6</sub> is a vinyl group (—CH=CH<sub>2</sub>), while in the case of silicone having —H in a part of the organic group or the vinyl-modified silicone, any of R<sub>1</sub> to R<sub>6</sub> is a vinyl group. Particularly, in the case of the vinyl-modified silicone, in addition to —H, at least one of R<sub>1</sub> to R<sub>6</sub> is a vinyl group. n, l and m each independently represents an integer of 1 or more decided appropriately according to the molecular weight of a releasing resin. Further, the atom groups of l and m parts are randomly polymerized. <sup>50</sup>

As other specific examples of vinyl modified silicones, the following modified silicones are illustrated.

One side end type



Both side end type



One side end + center type



-continued

(4)

Both side end + center type



As a preferred example, when the silicone of the above-mentioned formula (1) and the silicone of the above-mentioned formula (4) are mixed and undergo catalytic hardening, the reaction is schematically shown as follows.



When the above-mentioned multifunctional silicone is employed together, the main chain A contributes to the increase in the strength of a coated layer and the pendant B contributes to the improvement in releasing ability and excellent coated layer properties and releasing ability are accomplished at the same time.

As specific examples of the above-mentioned vinyl-modified silicones of the hardening reaction type, compounds shown in the following Table 1 are illustrated.

TABLE 1

| No. | Molecular Weight | Reactive Group | Position of Reactive Group | Reactivity Number     | Basic   | Silicone Skeleton    |
|-----|------------------|----------------|----------------------------|-----------------------|---------|----------------------|
| 45  | A                | 3400           | Vinyl group                | one side end          | 4/mole  | vinyl siloxane       |
|     | B                | 3400           | Vinyl group                | one side end          | 4/mole  | vinyl phenylsiloxane |
|     | C                | 7000           | Vinyl group                | one side end          | 4/mole  | vinyl siloxane       |
|     | D                | 7000           | Vinyl group                | one side end          | 13/mole | vinyl siloxane       |
|     | E                | 10000          | Vinyl group                | one side end          | 13/mole | vinyl siloxane       |
| 50  | F                | 3500           | Vinyl group                | both ends             | 13/mole | vinyl phenylsiloxane |
|     | G                | 3500           | Vinyl group                | both ends             | 32/mole | vinyl phenylsiloxane |
|     | H                | 7000           | Vinyl group                | both ends             | 13/mole | vinyl phenylsiloxane |
|     | I                | 17000          | Vinyl group                | both ends             | 13/mole | vinyl phenylsiloxane |
|     | J                | 3500           | Vinyl group                | one side end + center | 4/mole  | vinyl phenylsiloxane |
| 55  | K                | 7000           | Vinyl group                | one side end + center | 4/mole  | vinyl siloxane       |
|     | L                | 10000          | Vinyl group                | one side end + center | 4/mole  | vinyl siloxane       |
|     | M                | 22000          | Vinyl group                | one side end + center | 4/mole  | vinyl siloxane       |
|     | N                | 3500           | Vinyl group                | both ends + center    | 8/mole  | vinyl phenylsiloxane |
|     | O                | 7000           | Vinyl group                | both ends + center    | 8/mole  | vinyl phenylsiloxane |
| 65  | P                | 17000          | Vinyl group                | both ends + center    | 8/mole  | vinyl phenylsiloxane |



Namely, the releasing resin having a substitute excellent in compatibility with a resin for forming the releasing layer is employed. Because the compatibility of the releasing resin depends especially on the type and amount of the organic group other than the reactive group, the organic group can be replaced with a substitute good in compatibility with a resin for forming the releasing layer. Accordingly, in accordance with the type of the resin for forming the releasing layer, a substitute group good in the compatibility with the above-mentioned resin is selected and a releasing resin of which organic group is replaced with the group in a predetermined ratio. Thus, at the preparation of an ink composition for forming the releasing layer, the good compatibility is secured between the releasing resin and the ink composition in the resin for forming the releasing layer and the releasing resin becomes preferably compatible with the resin for forming the releasing layer. As a result, the releasing layer prepared by employing the ink composition for forming the releasing layer with which the releasing resin is uniformly mixed kneaded is also formed as a uniform layer and the releasing effect is exhibited uniformly over the whole layer without fluctuation.

As one example of the above-mentioned, the polyester resin is employed as the resin for forming the releasing layer and in contrast to this, is explained a case in which a silicone-based releasing resin is employed.



Further, in the above-mentioned formula, X represents a reactive group such as an amino group, an epoxy group, an isocyanato group, a carboxyl group, a hydroxide group or a vinyl group. R represents a methyl group or an organic group having an alkyl group other than the methyl group. l, m and n each independently represents an integer and groups of atoms in a part of l, m and n are copolymerized randomly.

Because for the polyester resin herein, for example, a phenyl group is a highly compatible substituent, a part of R is replaced with the phenyl group. The replacement ratio to the phenyl group, when R is a methyl group, is methyl group/phenyl group=95 to 5/5 to 95 and preferably 70 to 20/30 to 80.

As mentioned above, by employing any one having a substituent excellent in compatibility with a resin for forming the releasing layer as the releasing resin, compatibility of the resin for forming the releasing layer with the releasing resin in the composition for forming the releasing layer is improved to increase the pot life of the above-mentioned composition and no separation is caused. (3) Combination of any of those which decreases the equivalent of a reaction group or have the different equivalent in the case of the reaction hardening type releasing resin.

Namely, the releasing resin having the equivalent (=molecular weight/number of reaction groups per one molecule) of the reaction group of 300 or less, preferably in the range of 100 to 250 is employed. According to this, the number of reaction groups which the releasing resin has increases to improve the reactivity of the releasing resin at the formation of the releasing layer. As a result, the releasing layer is obtained which is hardened firmly in a short time.

In addition, among two types of reaction hardening type releasing resins, at least in one side, is employed a releasing resin composed of two or more of different equivalents of

the reaction group. According to this, reactivity of the releasing resin is considerably improved at the formation of the releasing layer. As a result, the releasing layer which is firmly hardened in a short time is obtained. Here, as an embodiment of a combination of two types of releasing resins employed at the formation of the releasing layer, case in which two types A and B of reaction effective type are employed;

- 10 (i) as B, one type of the equivalent of a reaction group is employed and as B, those having different equivalent of the group of two or more are combined.
- 15 (ii) as B, one type of the equivalent of a reaction group is employed and as A, those having different equivalent of the group of two or more are combined.
- 20 (iii) as A and B, both of each having the different equivalent of the reaction group of two or more are combined.

Coupling agents include, for example, those having a long chain alkyl group which may be substituted with a fluorine atom. The long chain alkyl groups in the above mentioned coupling agent includes, for example, those such as hexyl, isohexyl, octyl, decyl, lauryl, tridecyl, tetradecyl, pentadecyl, heptadecyl, octadecyl, nonadecyl, eicosyl, docosyl, tricosyl, pentacosyl, hexacosyl group, etc. or its fluorine substituted group and of these, the alkyl group having carbon atoms of 15 or more is preferred.

Those which are preferred as the above-mentioned coupling agents include silane coupling agents and titanium coupling agents, and are preferably employed, for example, hepta dec a fluor o de c yl trichlorosilane, hepta dec a fluor o de c yl trim thoxysilane, hepta dec a fluor o de c yl methyl dichlorosilane, hepta dec a fluor o de c yl methyl dimethoxysilane, octadecyl dimethyl chlorosilane, octadecyl triethoxysilane, 35 octadecyl trimethoxysilane, octadecyl methyl dichlorosilane, octadecyl methyl trimethoxysilane, isopropyl triisooctanoyl titanate, isopropyl (diethylpyrophosphate) titanate, isopropyl tristearoyl titanate, isopropyl tris (diethylphosphate) titanate, isopropyl dimethacrylisostearoyl titanate, etc.

Besides the incorporation of the above-mentioned coupling agent into the releasing layer, it may be individually employed as an organic solution to form a releasing layer on the surface of the releasing layer. In this case, a small amount of a resin binder so as not to hinder the accomplishment of the object of the present invention may be combined in the above-mentioned solution. As such the resin binder, the thermoplastic resin for forming the releasing layer can be employed, as it is, and when the above-mentioned thermoplastic resin has an active hydrogen group such as a hydroxyl group, it can appropriately be crosslinked by the addition of polyisocyanate and close contact properties and layer strength of the formed releasing layer can be improved. As another preferred resin binder, the resin having a urethane bond and/or a urea bond is illustrated. The resin having the urethane bond and/or the urea bond is to be prepared by the reaction between a compound comprising a multifunctional active hydrogen and polyisocyanate.

As the compound comprising the active hydrogen, there are illustrated various kinds of polyols and polyamines 60 having a low or high molecular weight. For example, there are illustrated ethylene glycol, diethylene glycol, triethylene glycol, polyethylene glycol, propylene glycol, dipropylene glycol, tripropylene glycol, polypropylene glycol, glycerin, pentaerythritol, bisphenol A, or ethylene oxide and/or propylene oxide addition compounds, for example, polymer or copolymer of a acryl monomer having a hydroxide group such as, for example, acrylpolyol, hydroxyethyl(meta)

acrylate, a vinyl resin containing a vinyl alcohol unit such as a polymer or copolymer of vinyl acetate, a polyvinyl acetal resin, a cellulose resin, etc. However, the present invention is not limited to those polyols. Furthermore, polyamines include low molecular weight and high molecular weight polyamines such as ethylenediamine, propylenediamine, triethylenediamine, tripropylenediamine, polyethylene polyamine, polyethylene imine, polyacrylamide, etc. polyamine, polyethyleneimine, polyacrylamide, etc.

In addition, as polyisocyanates employed if desired, there are illustrated various kinds of polyisocyanates employed widely in conventional polyurethane resins, polyurethane paints, polyurethane adhesives, etc., such as, for example, 2,4-tolylene diisocyanate (2,4-TDI), 2,5-tolylene diisocyanate (2,5-TDI), 4,4'-diphenylmethanediisocyanate (MDI), hexamethylenediisocyanate (HMDI), isophoronediisocyanate, triphenylmethanetriisocyanate, triphenylmethanetriisocyanate, tris(isocyanatephenyl) thiophosphate, lysinestertriisocyanate, 1,8-diisocyanate-4-isocyanatemethyloctane, 1,6,11-undecanetriisocyanate, 1,3,6-hexamethylenetriisocyanate, bicycloheptanetriisocyanate, burete bonded HMDI, isocyanate bonded HMDI, trimethylolpropane-TDI 3 mole addition compound or mixtures of thereof. The reaction of the compound containing a multifunctional active hydrogen as mentioned above with polyisocyanate may be carried out prior to, during or after the formation of the releasing layer. In the case prior to the formation, the reaction is desirably carried out so that the resin formed is not gelled. When the resin binder as described above is employed, it is preferred to use those in the range of 10 to 1,000 parts by weight per one weight part of the above-mentioned coupling agent.

As long chain alkyl compounds, there are illustrated, for example, alcohols, amines, carboxylic acids, epoxy compounds, silane coupling agents, titanium coupling agents, aluminum series coupling agents, etc. having a long chain alkyl group, for example, a hexyl, isohexyl, heptyl, octyl, decyl, lauryl, tridecyl, tetradecyl, pentadecyl, heptadecyl, octadecyl, nonadecyl, eicosyl, docosyl, tricosyl, pentacosyl, hexacosyl group, etc. Of these, the compounds having an alkyl group having carbon atoms of 15 or more are preferred.

Polyoxyalkylenepolyol is a general term for the following compositions (1), (2) and (3) and/or those reaction products.

- (1) active hydrogen compound, polyisocyanate and alkylene oxide
- (2) active hydrogen compound, polyisocyanate and long chain alkylisocyanate
- (3) active hydrogen compound, polyisocyanate and polymerizable monomer having a long chain alkyl group

As the above-mentioned active hydrogen containing compounds, those as described below are employed. Furthermore, oligomers terminated with polyisocyanate may be employed which have been previously prepared by reacting these active hydrogen compounds with polyisocyanate. As active hydrogen containing compounds, there are illustrated various kinds of polyols and polyamines having a low or high molecular weight. For example, there are illustrated ethylene glycol, diethylene glycol, triethylene glycol, polyethylene glycol, propylene glycol, dipropylene glycol, tripropylene glycol, polypropylene glycol, glycerin, pentaerythritol, bisphenol A, or ethylene oxide and/or propylene oxide addition compounds, for example, polymer or copolymer of a acryl monomer having a hydroxide group such as, for example, acrylpolyol, hydroxyethyl(meta) acrylate, a vinyl resin containing a vinyl alcohol unit such as a polymer or copolymer of vinyl acetate, a polyvinyl acetal resin, a cellulose resin, etc. However, the present invention

is not limited to those polyols. Furthermore, as polyamines, there are illustrated low molecular weight and high molecular weight polyamines such as ethylene diamine, propylene diamine, triethylene diamine, tripropylenediamine, polyethylene polyamine, polyethylene imine, polyacrylamide, etc. However, the present invention is not limited to those polyamines.

In addition, as polyisocyanates employed if desired, there are illustrated various kinds of polyisocyanates employed widely in conventional polyurethane resins, polyurethane paints, polyurethane adhesives, etc., such as, for example, 2,4-tolylene diisocyanate(2,4-TDI), 2,5-tolylene diisocyanate (2,5-TDI), 4,4'-diphenylmethanediisocyanate(MDI), hexamethylenediisocyanate(HMDI), isophoronediisocyanate, triphenylmethanetriisocyanate, tris(isocyanatephenyl) thiophosphate, lysinestertriisocyanate, 1,8-diisocyanate-4-isocyanatemethyloctane, 1,6,11-undecanetriisocyanate, 1,2,6-hexamethylenetriisocyanate, bicycloheptanetriisocyanate, burete bonded HMDI, isocyanate bonded HMDI, trimethylolpropane-TDI 3 mole-addition compound or mixtures of thereof. The added amount of those polyisocyanates vary according to the active hydrogen containing amount of the above-mentioned releasing polymer, amount of added active hydrogen containing compound, forming conditions of a releasing layer or releasing agent. In practice, the amount of 1.5 equivalent or less per one equivalent of the above-mentioned releasing polymer or active hydrogen of the active hydrogen-containing compound is generally employed.

The above-mentioned long chain alkyl isocyanates can be prepared by isocyanizing a long chain aliphatic amine. As examples of the long chain aliphatic amines, there are illustrated hexylamine, isohexylamine, heptylamine, octylamine, decylamine, laurylamine, tridecylamine, tetradecylamine, pentadecylamine, heptadecylamine, octadecylamine, nonadecylamine, eicosylamine, docosylamine, tricosylamine, pentacosylamine, hexacosylamine, etc. The long chain alkylisocyanates employed in the present invention are prepared by converting the amino group of those long chain alkyl amines to an isocyanate group. Of those long chain alkylisocyanates, those having 15 or more of carbon atoms, for example, octadecylisocyanate, etc. readily commercially available are particularly preferred.

The above-mentioned alkyl group containing addition polymerizable monomers include reaction products of addition-polymerizable unsaturated carboxylic acid such as acrylic acid, methacrylic acid, itaconic acid, maleic acid, etc. with long aliphatic alcohols or long chain aliphatic amine, esters of vinyl alcohols with long chain aliphatic acids. As carbon chains of the above-mentioned long chain alcohol, amine, carboxylic acid, etc. there are illustrated, for example, a hexyl, isohexyl, heptyl, octyl, decyl, lauryl, tridecyl, tetradecyl, pentadecyl, octadecyl, nonadecyl, eicosyl, docosyl, tricosyl, pentacosyl, hexacosyl group, etc. Of those long chain alkyl groups, those having 15 or more of carbon atoms, for example, alcohol, amine or carboxylic acid having a stearyl group, readily commercially available are particularly preferred.

Furthermore, the above-mentioned long chain alkyl group containing addition-polymerizable monomer may be individually polymerized or may be copolymerized together with other addition-polymerizable monomers. Particularly, when a polymer is allowed to react with polyisocyanate, preferably are copolymerized monomers having a group such as a hydroxyl group which reacts with an isocyanate group, for example, monomers subjected to ring-opening

15

addition of moles (1 to 10 moles) of ethylene oxide, propylene oxide or caprolactone to a terminal hydroxyl group of 2-hydroxyethyl(meta)acrylate, 2-hydroxypropyl(meta)acrylate, 2-hydroxyethyl(meta)acrylate. As the other copolymerizable monomers, for example, various kinds of general monomers such as other (meta)acrylic acid esters, various carboxylic esters, styrene, vinyl chloride, vinyl pyrimidine, etc. In the case of copolymerization with those other addition-polymerizable monomers, a ratio of the long chain alkyl group containing addition polymerizable monomer is preferably in the range of from 30 to 95 mole percent of the total copolymer and when employing the active hydrogen-containing monomer, the ratio is preferably in the range of 5 to 70 mole percent. When the ratio of the long chain alkyl group-containing addition-polymerizable monomer is less than the above range, the polymer obtained exhibit insufficient releasing properties.

As the above-mentioned alkylene oxides, there are illustrated, for example, ethylene oxide, propylene oxide, butylene oxide, etc. When these alkylene oxides undergo addition polymerization to the above-mentioned active hydrogen compounds, either individual polymerization or copolymerization may be carried out and any order of the addition may be employed. Furthermore, as catalysts employed during the addition polymerization, there are illustrated generally basic catalysts such as sodium methylate, sodium hydroxide, potassium hydroxide, lithium carbonate, etc. However, Lewis acid catalysts such as boron trifluoride and amine series catalysts such as trimethylamine or triethylamine are also useful and the addition amount may be the same as commonly used. As particularly preferred polyoxyalkylenepolyols, the following general formulas (A) to (E) are particularly illustrated.



16

-continued

(E)



(wherein R represents  $-\text{C}_2\text{H}_4$ ,



P represents  $-\text{CH}_2\text{CH}_3$ ,  $-\text{CH}_2\text{O}-(\text{RO})_n-\text{H}$  and  
 n is a numerical figure wherein number average molecular  
 weight is in the range of 200 to 5,000)

Organic polyisocyanates to enable the above-mentioned polyols to crosslink, include, for example, 2,4-tolylenediisocyanate (2,4-TDI), 2,6-tolylenediisocyanate (2,6-TDI), 4,4'-diphenylmethanediisocyanate (MDI), hexamethylenediisocyanate (HMDI), isophoronediisocyanate (IPDI), triphenylmethanetriisocyanate, triisocyanatephenylthiophosphate, lysinestertriisocyanate, 1,8-diisocyanate-4-isocyanatemethyloctane, 1,6,11-undecanetriisocyanate, 1,3,6-hexamethylenetriisocyanate, bicycloheptanetriisocyanate, further, those termed isocyanate adduct compounds such as buret bonded HMDI, isocyanate bonded HMDI, trimethylolpropane-TDI 3 mole addition compound or mixtures of thereof.

When the above-mentioned polyoxyalkylenepolyols are allowed to react with the above-mentioned polyisocyanates, both are preferably mixed for the reaction so that the base number of the organic polyisocyanate is in the region of 0.8 to 2.5 times to the terminal hydroxide group of polyoxyalkylenepolyol. Furthermore, when the reaction is accomplished in a short time, it is useful to employ a catalyst. The catalysts include, for example, organic metal catalysts such as dibutyl tin dilaurate (DBTDL), dibutyl tin diacetate (DBTA), phenyl mercury propionic acid salt, octanic acid lead, etc. or amine-based catalysts such as triethylenediamine, N,N'-dimethylpiperazine, N-methylmorpholine, tetramethylguanidine, triethylamine, etc. The above-mentioned polyurethane resin can be employed individually or as a mixture and further, it can be employed together with the other thermoplastic resins, for example, polyolefin series resins such as polypropylene, etc., halogenated polymers such as polyvinyl chloride, polyvinyl vinylidene, etc., vinyl polymers such as polyvinyl acetate, polyacryl ester, polyvinyl acetal, etc. polyester series resins such as polyethylene terephthalate, polybutylene terephthalate, etc., polystyrene series resins, polyamide series resins, copolymers of olefin such as ethylene or propylene, etc. with other vinyl monomer, ionomer, cellulose series resins such as cellulose diacetate, etc., polycarbonates, etc.

Particularly, in the present invention, it is preferred to add a releasing agent excellent in compatibility with a binder for the releasing layer. For example, when the vinyl chloride series resin is employed as a binder, it is preferred to employ a polyester-modified silicone resin together with it. As representative polyester-modified silicone resins, can be enumerated, for example, a copolymer of diol with dibasic acid or a block copolymer, that is, ring-opening polymer of polyester with dimethylpolysiloxane (including copolymers

in which both ends or one side end of dimethylpolysiloxane is blocked by the above-mentioned polyester part, or inversely, the above-mentioned polyester is blocked by dimethylpolysiloxane). Or a copolymer can be illustrated which is prepared by bonding polysiloxane to the side chain (dimethyl) while making the above-mentioned polyester a main chain. The added amount of those simply addition type silicone oils cannot be uniformly determined because it varies variously according to its kind. However, generally speaking, the amount is usually in the range of from 0.5 to 80 weight percent and preferably 10 to 50 weight percent of the solid component in the releasing layer.

In case that the post chelate dye is incorporated in the ink layer of the ink sheet, it is preferable that a metal ion-containing compound which is capable of chelate reacting with the post chelate dye is incorporated in the thin film material. The metal ion-containing compound works as a dye fixer. The metal ion-containing compound may be incorporated in a layer containing the metal ion-containing compound provided independently, or in the releasing layer. In case that the metal ion-containing compound is incorporated in an independent layer binder therefor is selected from those for ink layer, which will be mentioned later. An amount of the metal ion-containing compound is preferably 0.01 to 40 wt %, more preferably 0.1 to 20 wt % with regard to the solid component of the layer.

In the present invention, the ink sheet is composed of at least a support and an ink sheet provided thereon and the above-mentioned ink layer comprises a thermally transferable dye. The post chelate dye is preferably employed as the dye.

As the support for the ink sheet, there is no particular limitation as far as it exhibits good dimensional stability and withstands heat at recording with a heat-sensitive head can be employed. Practically, for example, the same thin film material as mentioned above are employed.

As the binder of the ink layer, there can be illustrated, for example, cellulose series resins such as a cellulose addition compound, cellulose ester, cellulose ether, etc., polyvinyl acetal resins such as polyvinyl alcohol, polyvinyl formal, polyvinyl acetoacetal, polyvinyl butyral, etc., vinyl series resins such as polyvinylpyrrolidone, polyvinyl acetate, polyacrylamide, styrene series resins, poly(meta)acrylic acid series esters, poly(meta)acrylic acid, (meta)acrylic acid copolymer, rubber series resins, ionomer resins, olefin series resins, polyester resins, etc. Of these resins, the polyvinyl butyral, polyvinyl acetoacetal or cellulose series resins having excellent preservation quality are preferred.

As the binder of the ink layer, resins mentioned below can be employed.

In Japanese Patent Publication Open to Public Inspection No. 5-78437 there are illustrated reaction products of isocyanates with compounds having an active hydrogen selected from polyvinyl butyral, polyvinyl formal, polyterpolyol and acrylpolyol, the above-mentioned reaction products in which isocyanates are diisocyanates or triisocyanates and the above-mentioned reaction products of 10 to 200 weight parts for 100 weight parts of the active hydrogen-containing compound; organic solvent-soluble high polymer in which intramolecular hydroxide groups in a natural and/or semi-synthesized water-soluble high polymer are esterified and/or urethanized, as the natural and/or semi-synthesized water-soluble high polymers, starch which is a polymer having an  $\alpha$ -1,4-glucosido bond of  $\alpha$ -glucose, water-soluble derivative of cellulose which is a polymer having a  $\beta$ -1,4-glucosido bond of  $\beta$ -glucose, alginic acid which is a polymer having a  $\beta$ -1,4-glucosido bond of a pyranose ring, maltotriose which is a trimer of glucose, pullulan which is a water-soluble polysaccharide bonded repeatedly with a 1,6 bond of a  $\alpha$ -D-1,6-glucose, dextran

which is a polymer composed of D-glucopyranose as a unit prepared from sugar, curdran which is a straight chain  $\beta$ -1,3-glucan having a  $\beta$ -glucosido bond at 1,3 bond of D-glucose; cellulose acetates having a degree of acetylation of 2.4 or more and degree of total replacement of 2.7 or more which are described in Japanese Patent Publication 3-264393; vinyl resins such as polyvinyl alcohol ( $T_g=85^\circ C.$ ), polyvinyl acetate ( $T_g=32^\circ C.$ ), vinyl chloride/vinyl acetate copolymer ( $T_g=77^\circ C.$ ), etc. polyvinyl acetal series resins such as polyvinyl butyral ( $T_g=84^\circ C.$ ), polyvinyl acetoacetal ( $T_g=110^\circ C.$ ), etc., vinyl series resins such as polyacrylamide ( $T_g=165^\circ C.$ ), polyester resins such as aliphatic polyester ( $T_g=130^\circ C.$ ), etc. and the like; reaction products of isocyanates with polyvinyl butyral in which the weight of contained part of the vinyl alcohol is from 15 to 40 percent, described in Japanese Patent Publication Open to Public Inspection No. 7-52564, the above-mentioned reaction products in which the above-mentioned isocyanates are diisocyanates or triisocyanates, specifically, para-phenylenediisocyanate, 1-chloro-2,4-phenylenediisocyanate, 2-chloro-1,4-phenylenediisocyanate, 2,4-toluenediisocyanate, 2,6-toluenediisocyanate, hexamethylenediisocyanate, 4,4'-biphenylenediisocyanate, 4,4',4"-trimethyl-3,3',2-triisocyanate-2,4,6-triphenylcyanate, etc.; phenylisocyanate-modified polyvinyl acetal resins of the formula I described in Japanese Patent Publication Open to Public Inspection No. 7-32742; compounds obtained by hardening compositions consisting of one of isocyanate reactive cellulose or isocyanate reactive acetal resin, and one resin selected from isocyanate reactive acetal resin, isocyanate reactive vinyl resin, isocyanate reactive acrylic resin, isocyanate reactive phenoxy resin and isocyanate reactive styrol resin, and a polyisocyanate compound, described in Japanese Patent Publication Open to Public Inspection No. 6-155935; polyvinyl butyral resins (having preferably molecular weight of 60,000 or more, glass transition temperature of  $60^\circ C.$  or higher, more preferably  $70^\circ C.$  or higher and  $110^\circ C.$  or lower, weight percent of vinyl alcohol part of 10 to 40 percent of polyvinyl butyral resin, preferably from 15 to 30 percent); acryl-modified cellulose series resins, as the cellulose series resins, cellulose series resins (preferably ethylcellulose) such as ethylcellulose, hydroxyethylcellulose, ethylhydroxycellulose, hydroxypropylcellulose, methylcellulose, cellulose acetate, cellulose butyrate, etc. As organic solvents employed in the modification of the above-mentioned cellulose series resins with acrylic resins, there are provided, for example, ester series solvents such as methyl formate, ethyl formate, ethyl acetate, butyl acetate, etc., ketone series solvents such as acetone, methyl ethyl ketone, methyl isobutyl ketone, cyclohexanone, isophoron, etc., hydrocarbon series solvents such as toluene, benzene, xylene, etc., ether series solvents such as n-butyl ether, etc., and the cellulose series resins are preferably employed at a concentration of about 5 to about 50 weight percent. The above-mentioned various binders are employed individually or in combination of two or more thereof.

A reactive dye is used as the thermally diffusible dye to be contained in the ink layer. The reactive dye is a dye capable of forming an image by reaction of a precursor of the dye contained in the ink layer with the dye fixing agent by thermal transfer. A combination of a post-chelating dye and a metal source is preferably used in view of preferable image stability, although known reactive dye, including the foregoing, can be used. Known various compounds are usable as the post-chelating dye without any limitation as long as the dye can be thermally transferred. In concrete, cyan dyes, magenta dyes and yellow dyes described in, for example, described in JP O.P.I. Nos. 59-78893, 59-109349, 94974, 4-97894 and 4-89292 are usable.

19

Among these dyes, one capable of forming a di-dentate chelate with the metal source is preferable used. Examples of such the dye are ones represented by the following Formula 1.

5  
Formula 1

In the above formula, A is a group of atoms having a group or an atom each a capable of forming a di- or more dentate chelate, Y is a group of atoms necessary to form an aromatic carbon ring or heterocyclic ring, R<sub>1</sub>, R<sub>2</sub> and R<sub>3</sub> are each independently a hydrogen atom, a halogen atom or a mono-valent substituent. n is 0, 1 or 2. Y is preferably a group of atoms necessary to form a 5- or 6-member aromatic carbon ring or heterocyclic ring, which may have a substituent. 15

The group represented by X is preferably one represented by the following Formula 2. 20

25  
Formula 2

In the above formula, Z is a group of atoms necessary to 30 form an aromatic nitrogen-containing heterocyclic ring having a substituent containing a nitrogen atom capable of forming a chelate.

Examples of such the ring include a benzene ring, a 35 pyridine ring, a pyrimidine ring, a furan ring, a thiophene ring, a thiazole ring, an imidazole ring and a naphthalene ring. These rings each may be condensed with a carbon ring such as a benzene ring or a heterocyclic ring such as a pyridine ring.

Examples of the substituent of such the ring include an 40 alkyl group, an aryl group, an acyl group, an amino group, a nitro group, a cyano group, an acylamino group, an alkoxy group, a hydroxyl group, an alkoxy carbonyl group and a halogen atom. These group each may have a substituent thereof.

Example of the halogen atom represented by R<sub>1</sub>, R<sub>2</sub> or R<sub>3</sub> include a fluorine atom and a chlorine atom, and those of a 45 mono-valent substituent represented by R<sub>1</sub>, R<sub>2</sub> or R<sub>3</sub> include an alkyl group, an alkoxy group, a cyano group and an alkoxy carbonyl group.

Groups represented by the following Formula 3, 4, 5 or 6 are preferable as the group represented by X=.

55  
Formula 3

20

-continued

Formula 4



Formula 5



Formula 6



In the above-mentioned formulas, R<sub>4</sub> and R<sub>5</sub> are each a 30 hydrogen atom, a halogen atom such as a fluorine atom, chlorine atom and a bromine atom, or a mono-valent substituent such as an alkyl group, an aryl group, an amino group, a nitro group, a cyano group, an acylamino group, an alkoxy group, a hydroxyl group, and an alkoxy carbonyl group.

Examples of the post-chelating dye are shown below. 50

(1)



**21**

-continued



(2)

**22**

-continued



5

10

15

20

25

30

35

40

45

50

55

60

65

(6)

(7)

(8)

(9)

23

-continued



The chemical structure of Caffeine (1,3,7-trimethylxanthine) is shown. It features a purine ring system with three methyl groups (CH<sub>3</sub>) attached to the 1, 3, and 7 positions. The purine ring is substituted with a 2-phenyl group (a phenyl ring attached to the 6-position) and a 1-(diethylamino)ethyl group (a CH<sub>2</sub>CH<sub>2</sub>N(C<sub>2</sub>H<sub>5</sub>)<sub>2</sub> group attached to the 8-position).

24

-continued

(14)



(11)



(12)



(13) 50



(15)

(16)

(17)

**25**

-continued



(18)

**26**

-continued



(22)



(23)



(19)



(24)



(20)



(25)



(21)



(27)



-continued



The post-chelating dye is usually used in an amount of from 10% to 80% by weight of the whole compositions contained in the area containing the post chelate dye, even though the content of the post-chelating dye may be changed depending on the property of the dye, the solubility of the dye in the binder or the purpose of use.

Various kinds of additive other than the above-mentioned may be optionally further added to the ink layer. The additives include the foregoing mold releasing agent such as a silicone compound including reaction hardenable type, a silicone-modified resin, a fluorized resin, a surfactant and a wax, a filler such as a fine metal powder, a silica gel, a metal oxide, carbon black, and a resin powder, a hardening agent capable of reacting with the binder, for example, a irradiation reactive compound such as an isocyanate compound, an acryl compound and an epoxy compound.

Another layer may be further provided on the support of the ink sheet. For example, an over-coat layer may be provided on the surface of the ink layer to prevent adhesion or blocking with the image receiving layer caused by fusion and transfer of dye to the back side of another sheet.

A subbing layer may be provided on the support of the ink sheet for improving an adhesion ability of the support to the ink layer and for preventing transfer of the dye precursor to the support. Furthermore, an anti-sticking layer may be provided on the back side, opposite to the ink layer provided side, for preventing fusion adhesion and sticking of the thermal head to the support and formation of a wrinkle of the support. The thickness of the over-coat layer, the subbing layer and the anti-sticking layer are each ordinary from 0.1  $\mu\text{m}$  to 1  $\mu\text{m}$ .

The ink sheet can be manufactured in such a way that an ink layer-preparing coating liquid is prepared by dissolving or dispersing the above-mentioned various compositions composing an ink layer to a solvent and the resulting is coated on the surface of a support for the ink sheet employing, for example, a gravure printing process and dried. The thickness of the formed ink layer is generally in the range of from 0.2 to 10  $\mu\text{m}$  and preferably in the range of from 0.3 to 3  $\mu\text{m}$ .

The ink layer of the present invention may incorporate a low molecular substance having a melting point of 50 to 150° C. as a sensitizer. The sensitizer having the melting point of lower than 50° C. is not preferred because it tends to move to the surface of the ink layer and on the other hand, the sensitizer having the melting point of higher than 150° C. is not preferred because the sensitizing action decreases sharply.

Furthermore, the molecular weight of the sensitizer is preferably in the range of 100 to 1,500. The sensitizer having the molecular weight of less than 100 is not preferred because its melting point is generally lower than 50° C. On the other hand, the sensitizer having the molecular weight of larger than 1,500 is also not preferred because the fusion sharpness is lost and the sensitizing action becomes insufficient.

Furthermore, the used amount of the above-mentioned sensitizer is preferably in the range of 1 to 100 parts by weight per 100 parts by weight of the binder employed to form the ink layer. The used amount of less than 1 part by weight is not preferred because no satisfactory sensitizing action is obtained. On the other hand, the used amount exceeding 100 parts by weight is not preferred because the thermal resistance of the ink layer decreases.

As sensitizers such as mentioned above, those having a low molecular weight are available as far as those have a melting point of 50 to 150° C. However, as those preferred, there are illustrated thermoplastic oligomers, for example, various kinds of oligomers such as polyurethane oligomer, polystyrene oligomer, polyester oligomer, polyacryl oligomer, polyethylene oligomer, polyvinyl chloride oligomer, polyvinyl acetate oligomer, ethylene/vinyl acetate copolymer oligomer, ethyleneacryl copolymer oligomer, polyoxethylene oligomer, polyoxypolyethylene oligomer, polyoxypolyethylenepropylene oligomer, etc., fatty acids such as myristic acid, palmitic acid, margaric acid, stearic acid, arachic acid, montanic acid, etc., fatty acid amides such as caproic acid amide, caprylic acid amide, lauric acid amide, stearic acid amide, oleic acid amide, eicosanic acid amide, etc., fatty acid esters such as methyl behenate, pentadecyl palmitate, hexacocyl stearate, [1,4-phenylenebis (methylene)]bisdimethyl carbamate, etc., and aromatic compounds such as 1,4-dicyclohexylbenzene, benzoic acid, aminobenzophenone, dimetylterephthalate, fulorantene, phenols, naphthalenes, phenoxyres, various waxes, etc.

Image receiving sheet is described below.

Image receiving sheet comprises a support and an image receiving layer provided on the support.

The support of the image receiving sheet preferably possesses such a mechanical strength that keeps image receiving layer and is capable of handling when it is heated since the sheet is heated at the dye transfer process.

35 Examples of raw material for the support includes condenser paper, glassine paper, parchment paper, synthesized paper such as polyolefin paper and polystyrene paper, high quality paper, art paper, coated paper, cast-coated paper, wall paper, back reinforce paper, synthesized resin or emulsion sintered

40 paper, synthesized gum sintered paper, synthesized resin incorporated paper, cardboard, cellulose fiber paper, films such as polyester, polyacrylate, polycarbonate, polyurethane, polyimide, polyetherimide, cellulose derivative, polyethylene, ethylene-vinylacetate copolymer,

45 polypropilene, polystyrene, acryl, polyvinylchloride, polyvinilidenechloride, polyvinylalcohol, polyvinylbutyral, nylon, polyetheretherketon, polysulfon, polyethersulfon, tetrafluoroethylene, perfluoroalkylvinylether, polyvinylfluoride, tetrafluoroethylene ethylene, tetrafluoro-

50 ethylene hexafluoropropylene, polychlorotrifluoroethylene and polyvinylidenefluoride, white opaque film prepared by these synthesized resin by adding pigments or filler (representative examples can include titanium white, magnesium carbonate, zinc oxide, barium sulfate, silica talc, clay, calcium carbonate etc.) and formed sheet.

A laminated substance of combination of the above mentioned material is also applicable to the support. Representative examples include a synthesized paper of combination of cellulose fiber paper and synthesized paper or cellulose fiber paper and plastic film. The above mentioned material may be laminated on the synthesized paper or the plastic film to separate a function such as cushion characteristics and thermal conductivity. Thickness of the support is usually 10 to 300  $\mu\text{m}$ . Various primer processing or corona discharge processing may be preferably carried out when the adhesive strength is poor between the support and a layer provided thereon.

The image-receiving layer accepts a dye which is diffused upon heating from the ink layer of the ink sheet. The image-receiving layer is basically composed of a binder which accepts and immobilize the diffused dye to form a dye image and additives if necessary. As a method to form the image-receiving layer on the surface of the support, a coating method can be illustrated in that a coating liquid is prepared by dispersing or dissolving components forming the image-receiving layer and coat dried on the surface of the above-mentioned support, or a laminating method can be illustrated in that a mixture containing components forming the above-mentioned image-receiving layer is laminated on the surface of the support employing melt extrusion. The thickness of the image-receiving layer formed on the surface of the support is usually in the range of from 0.5 to 50  $\mu\text{m}$  and preferably from 1 to 20  $\mu\text{m}$ .

As the binder for an image-receiving layer, there can be employed binders such as vinyl chloride series resins, polyester series resins, polycarbonate series resins, acryl series resins, polyvinyl acetal series resin and various heat resisting resins. There is no restriction for the selection of the binder. In view of image preservation quality, etc., polyvinyl acetal resins or vinyl chloride series resin are preferred. As the above-mentioned polyvinyl acetal series resins, there can be illustrated polyvinyl acetal resins, polyvinyl acetoacetal resins, polyvinyl butyral resins, polyvinyl formal resins, etc. As the above-mentioned vinyl chloride series resins, copolymers of polyvinyl chloride resin and vinyl chloride can be included. As the vinyl chloride copolymers, there can be provided a copolymer of vinyl chloride containing vinyl chloride of 50 mole percent or more as a monomer unit with the other co-monomer. In addition to the above-mentioned polyvinyl acetal series resins and vinyl chloride series resins, the polyester series resins can be suitably employed as the image-receiving layer for thermal transfer. The polyester series resins can include, for example, polyethylene terephthalate, polybutylene terephthalate and compounds described in Japanese Patent Application Open to Public Inspection Nos. 58-188659 and 62-244696. In addition, as the polycarbonate series resins, for example, various kinds of compounds described in Japanese Patent Publication Open to Public Inspection No. 62-169694 can be included. As the acryl series resins, for example, polyacryl ester can be included. As heat-resisting resins, various kinds of known heat-resisting resins can be employed, as far as they exhibit good heat resistance, no extremely low softening point or glass transition point (Tg), appropriate compatibility with the above mentioned vinyl chloride series resins and substantially colorlessness. "Heat resistance" mentioned herein means that during the storage at high temperatures, a resin itself causes no coloration such as yellow stain and no extreme degradation of the physical strength. The softening point of the above-mentioned heat resisting resin is preferably in the range of from 30 to 200° C. and specially, its Tg is preferably from 50 to 150° C. The softening point of less than 30° C. is not preferred because the ink sheet and the image-receiving layer may be fused each other during thermal dye transfer. The softening point of 200° C. or higher is not preferable because sensitivity of the image-receiving layer decreases. As heat resisting resins meeting the above-mentioned requirements, phenol resin, melamine resin, urea resin ketone resin, etc. are illustrated. However, of them, urea aldehyde resin and ketone resin are particularly preferred. The urea aldehyde resin is prepared by condensation between urea and aldehydes (mainly, formaldehyde) and the ketone resin is prepared employing the condensation reaction between ketone and formaldehyde.

As the binder of the image-receiving layer, resins mentioned below can be further employed.

Polyolefin such as polypropylene, polyvinyl halide other than those mentioned above such as polyvinilidnechloride, vinyl polymer other than those mentioned above such as polyvinyl acetate, polystyrene resins, polyamide resins, copolymer resins of olefin such as ethylene and propylene and other vinyl monomer, ionomer, cellulose resins such as cellulose diacetate, polyurethane resins, polyimide resins, and epoxy resins.

Combination of a polycarbonate resin with an aromatic polyester resin described in Japanese Patent Publication Open to Public Inspection No. 5-246152; polyvinyl acetal series resins having a carboxyl group, the above-mentioned polyvinyl acetal series resins in which a component constructing the above-mentioned carboxyl group is an addition polymerizing monomer having a carboxyl group and resins in which the number of monomer units having the above-mentioned monomer is in the range of from 0.5 to 20 percent by weight disclosed in Japanese Patent Publication Open to Public Inspection No. 5-246151; vinyl chloride copolymer resins having an epoxy group described in Japanese Patent Publication Open to Public Inspection No. 5-246150; random-co-polycarbonate resins described in Japanese Patent Publication Open to Public Inspection No. 5-131758; polyester resins in which at least one of a diol component and an acid component contains an aliphatic cyclic compound and polyester resins in which the aforesaid aliphatic cyclic compound is tricyclodecane dimethanol, cyclohexanedicarboxylic acid, cyclohexane dimethanol or cyclohexanediol (employing the aforesaid resin, resistance such as light resistance, finger mark resistance, plasticity resistance of an image is improved) described in Japanese Patent Publication Open to Public Inspection No. 5-64976; polyamide resins described in Japanese Patent Publication Open to Public Inspection No. 4-299187; and resins having a molecular weight of the aforesaid resin in the range of from 5,000 to 20,000 and a softening point of from 50 to 170° C. described in Japanese Patent Publication Open to Public Inspection No. 4-299187; hydrophobic resins composed of hydrophobic resin solution described in Japanese Patent Publication Open to Public Inspection No. 4-347690; polyamide resins having an amine value of 3 or less, the above-mentioned polyamide resins having a molecular weight in the range of 5,000 to 20,000 and a softening point of 50 to 170° C. and the above-mentioned polyamide resins having an acidic component selected from dimer acid, propionic acid, adipic acid or azelaic acid described in Japanese Patent Publication Open to Public Inspection No. 4-299188; polyurethane resins and polyester resins described in Japanese Patent Publication Open to Public Inspection No. 4-299184; high molecular substances having coating layer forming or film forming capability, the above-mentioned substances and hardened substances having compositions containing B1 and/or B2 component described in Japanese Patent Publication Open to Public Inspection No. 4-223194; synthetic resins described in Japanese Patent Publication Open to Public Inspection No. 4-131287; urethane-modified polyester resins described in Japanese Patent Publication Open to Public Inspection No. 4-43082; vinyl chloride/vinyl acetate copolymers having an average degree of polymerization of 400 or less described in Japanese Patent Publication Open to Public Inspection No. 4-135794; acid resins having an acid value of 2 or more such as, for example, those having an ester bond, for example, (a) polyester resins, polyacrylate resins, polycarbonate resins, polyvinyl acetate resins, styreneacrylate resins, vinyltoluene acrylic resins, (b) those hav-

ing a urethane bond, for example, polyurethane resins, etc., (c) those having amide bond, for example, polyamide resins (nylon), (d) those having a urea bond, for example, urea resins, etc., (e) those having a high polar bond, for example, polycaprolactone resins, polystyrene resins, polyacrylonitrile resins, etc. (of these, polyester series resins are particularly preferred) described in Japanese Patent Publication Open to Public Inspection No. 2-107485; thermoplastic resins and reaction products of at least two or more of compounds (amino resins having a melamine skeleton, urea skeleton, benzoguanamine skeleton and isocyanates, etc.) having a reactive functional group (amino resins having a melamine skeleton, urea skeleton, benzoguanamine skeleton and isocyanates) described in Japanese Patent Publication Open to Public Inspection No. 2-107485; thermoplastic resins having a number average molecular weight of 15,000 or less (which are excellent in rapid drying during production, and peeling properties from a heat transfer sheet during image formation, chromogenic density and definition) and as the aforesaid thermoplastic resins, vinyl chloride acrylstyrene copolymers (vinyl chloride acrylstyrene copolymers, vinyl chloride vinyl acetate acrylstyrene copolymers, vinyl chloride vinyl acetate styrene copolymers, vinyl chloride butylacrylstyrene copolymers, vinyl chloride butylacryl copolymers, vinyl chloride methacrylstyrene copolymers, vinyl chloride vinyl acetate methacrylstyrene copolymers, vinyl chloride butylacrylmethacrylstyrene copolymers, vinyl chloride vinyl acetate butylacrylmethacrylstyrene copolymers, etc.) in an amount of 5-100 weight percent of the image receiving layer described in Japanese Patent Publication Open to Public Inspection No. 7-40670; aldehyde-modified vinyl alcohol resins and polyester resins having a number average molecular weight of 10,000 or less (advantages: improvements in durability of image density, light resistance, finger print resistance, thermoplasticity, etc.), the above-mentioned polyester resins in which aldehyde modification ratio of the aldehyde-modified vinyl alcohol resin is between 30 and 50 percent, the above-mentioned polyester resins having the aldehyde-modified vinyl alcohol resin of an average degree of polymerization of 200 to 3,000, the above-mentioned polyester resins in which one part of polyol component and/or acid component is a aliphatic cyclic compound, the above-mentioned polyester resins in which the aldehyde modification is of formalin, acetaldehyde, butyraldehyde (acetaldehyde or butyl aldehyde is particularly preferred.) described in Japanese Patent Publication Open to Public Inspection No. 5-270151; resins having a tensile strength of 200 kg/cm<sup>2</sup> or more (advantages: prevention of crack formation of an image-receiving layer, for example, polyester series resins, polyurethane resins, butyral series resins, polyolefin series resins such as polypropylene, etc., polyvinyl chloride, vinyl chloride-vinyl acetate copolymer series resins, ionomer, cellulose series resins such as cellulose diacetate, etc. polycarbonates, etc. (those which are particularly preferred are the polyester series resins and vinyl chloride-vinyl acetate copolymer series resins) described in Japanese Patent Publication Open to Public Inspection No. 6-115272; mixtures of polyvinyl alcohol and synthetic resin emulsion having a glass transition temperature of -100 to 20° C. and a polar group described in Japanese Patent Publication Open to Public Inspection No. 6-79974; mixtures of an aqueous dispersion of polyester resin which is insoluble or hardly soluble to a solvent and an aqueous dispersion of a thermoplastic resin other than the above-mentioned polyester resin described in Japanese Patent Publication Open to Public Inspection No. 6-79974; reaction

products of polyalkylene polyols with organic polyisocyanates described in Japanese Patent Publication Open to Public Inspection No. 6-15966; reaction products of polyester series resins with polyisocyanates described in Japanese Patent Publication Open to Public Inspection Nos. 58-215398, 61-199997, 2-178089 and 2-86494; reaction products of vinyl chloride-vinyl acetate copolymers having an active hydrogen with polyisocyanates described Japanese Patent Publication Open to Public Inspection in Nos. 1-160681, 1-123794 and 3-126587; thermoplastic resins having a hydroxide group, for example, polyvinyl acetal resins, the above-mentioned polyvinyl acetal resins in which the amount of polyvinyl alcohol unit is from 5 to 50 weight percent, vinyl chloride-vinyl acetate copolymers, the above-mentioned vinyl chloride-vinyl acetate copolymers in which the containing amount of polyvinyl alcohol unit is from 1 to 30 weight percent, polyesters, partially saponified polyvinyl acetate, partially or completely saponified compounds of vinyl chloride-vinyl acetate copolymers, acryl resins, polyurethane resins, etc., those which are particularly preferred are the polyvinyl acetal resins and vinyl chloride-vinyl acetate copolymers, preferred polyvinyl acetal resins are polyvinyl formal resins, polyvinyl acetoacetal resins and vinyl butyral resins (advantages: bridged products composed of the above-mentioned resin with a crosslinking agent are excellent in releasing ability and excellent in chromogenic density, definition, various durability and anti-embossing properties.) described in Japanese Patent Publication Open to Public Inspection No. 6-8646; polyvinyl acetal resins in which the containing amount of polyvinyl alcohol unit is 10 weight percent or more (or from 10 to 50 weight percent, the above-mentioned polyvinyl acetal resins having a degree of polymerization of 100 to 10,000, etc. described in Japanese Patent Publication Open to Public Inspection No. 5-294076.

Furthermore, in the case of the formation of the image-receiving layer, the above-mentioned resins may be crosslinked or hardened by radiation rays, heat, moisture, catalysts, etc. employing the reactive points (when there is no reactive point, it is rendered to the resin.) In the case, radiation ray active monomer such as epoxy or acryl and the crosslinking agent such as isocyanate may be utilized and those monomers and crosslinking agents may be added to the image-receiving layer as they are or may be enveloped in micro-capsules.

The image-receiving layer may comprise a metal ion-containing compound which is capable of forming a metal chelate with a dye in addition to a binder. When the metal source is incorporated in the image-receiving layer and a chelatable dye (hereinafter referred to as a "post chelate dye") with the metal source is employed as a dye incorporated in the dye-containing region of the ink sheet, the formed dye image may exhibit excellent advantages of high transferred density, high image preservation quality and especially, penetration resistance.

As the metal source, inorganic or organic salts of metal ions and metal complexes are illustrated and of those, organic acid salts or complexes are preferred. As the metal, single valent or polyvalent metals in the I to VIII Group in the Periodic Table are illustrated and of these, Co, Cr, Cu, Fe, Mg, Mn, Mo, Ni, Sn, Ti and Zn are preferred and Ni, Cu, Cr, Co and Zn are particularly preferred. Specific examples of the metal source include  $Ni^{2+}$ ,  $Cu^{2+}$ ,  $Cr^{2+}$ ,  $Co^{2+}$ , and  $Zn^{2+}$ , and salts of aliphatic group such as acetic acid, stearic acid, etc. or salts of aromatic carboxyl acids such as benzoic acid, salicylic acid, etc. Furthermore, complexes represented by the following general formula (1) are particularly pre-

ferred which can be consistently added to the image-receiving layer and are substantially colorless.



General formula (1)

In the general formula (1), M represents a metal ion, and represents preferably  $Ni^{2+}$ ,  $Cu^{2+}$ ,  $Cr^{2+}$ ,  $Co^{2+}$  or  $Zn^{2+}$ .  $Q_1$ ,  $Q_2$  and  $Q_3$  each independently represents a coordination compound which can coordinate with a metal ion and each of those may be the same or different. The coordinated compounds may be selected from those described in "Chelate Science (5)" (Nankodo).  $L^-$  represents an organic anion group which includes specifically tetraphenyl boron anion, alkylbenzene sulfonic acid anion, etc. X represents 1, 2 or 3; Y represents 1, 2 or 0 and Z represents 1 or 0. These are determined according to 4-ligand coordination or 6-ligand coordination in the complex represented by the general formula (1) or according to the number of ligands of  $Q_1$ ,  $Q_2$  and  $Q_3$ . P represents 1 or 2. As an specific example of this kind of the metal source, there may be illustrated those described in U.S. Pat. No. 4,987,049 or compounds No. 1 through No. 99 described in JP O.P.I. No. 9-39423.

The added amount of the metal source is preferably in the range of from 5 to 80 weight percent of the binder of the image-receiving layer and more preferably in the range of from 10 to 70 weight percent of the binder of the image-receiving layer. The excessively added amount of the metal source in the image-receiving layer is not preferred because of the appearance of metal source color in the background of the image receiving element.

To the image-receiving layer may be added a releasing agent, antioxidant, UV absorber, light stabilizing agent, filler, pigment, etc. Furthermore, a plasticizer as a sensitizer, heat solvent, etc. may be added.

The releasing agent can improve peeling properties of the ink layer of the ink sheet and the image-receiving layer of the image-receiving element. As this kind of the releasing agent, there are illustrated silicone oil (including those termed silicone resins); solid wax such as polyethylene wax, polypropylene wax, amide wax, Teflon powder, etc.; silicate compounds or those composite compounds; fluorine series or phosphoric acid ester series surface active agents; coupling agents; long chain alkyl compounds; polyoxyalkyl polyols, etc., and of these, the silicone oil is preferred.

As the UV absorbers, those which function to absorb ultraviolet rays incident to dye images and are capable in thermal transfer are practiced. For example, there can be employed compounds described in Japanese Patent Publication Open to Public Inspection Nos. 59-158287, 63-74686, 63-145089, 59-196292, 62-229594, 63-122596, 61-283595, 1-204788, etc. and compounds known in the art as those which improve the durability of images in photography and the other image recording materials. The mixing ratio by weight of a binder to a UV absorber is preferably in the range of 1:10 to 10:1 and more preferably in the range of 2:8 to 7:3.

The antioxidants can include those described in Japanese Patent Publication Open to Public Inspection Nos. 59-182785, 60-130735, 1-127387 and compounds known in the art which improve the durability of images in photography and the other image recording materials. UV absorbers and light stabilizers, can include compounds described in Japanese Patent Publication Open to Public Inspection Nos. 59-158287, 63-74686, 63-145089, 59-196292, 62-229594, 63-122596, 61-283595, 1-204788, etc. and compounds known in the art which improve image durability in photography and the other image recording materials.

As fillers, inorganic fine particles or organic resin particles can be illustrated. The inorganic fine particles can include silica gel, calcium carbonate, titanium oxide, acid clay, activated clay, alumina, etc. The organic fine particles can include fluororesin particles, guanamine resin particles, acrylic resin particles, silicone resin particles, etc. The added amount of those inorganic or organic resin particles, though it varies according to specific gravity, is preferably in the range of from 0.1 to 70 weight percent. As pigments, representative examples can include titanium white, calcium carbonate, zinc oxide, barium sulfate, silica talc, clay, kaolin, activated clay, acid clay, etc.

As plasticizers, there can be illustrated phthalic acid esters (for example, dimethyl phthalate, dibutyl phthalate, dioctyl phthalate, didecyl phthalate, etc.), trimellitic acid esters (for example, octyl trimellitate, isononyl trimellitate, isodecyl trimellitate, etc.), pyromellitic acid esters such as octyl pyromellitate, adipic acid esters, etc. Further, because the excessive addition of the plasticizer degrades the image preservation quality, the added amount of the plasticizer is generally in the range of 0.1 to 30 percent by weight of the binder of the image-receiving layer.

On the back side of the image receiving element, a slipping back layer may be provided.

When the slipping back layer is provided on the back side of the image-receiving element, an employed resin carries preferably low dyeability. Resins such as those, in practice, can include acrylate series resins, polystyrene series resins, polyolefin series resins, polyamide series resins, polyvinyl butyral, polyvinyl alcohol, cellulose acetate resins, etc.

Furthermore, amorphous polyolefin resins can be employed which are described in Japanese Patent Publication Open to Public Inspection No. 7-186557. In addition to those, hardened resins which are prepared by hardening polyvinyl butyral, melamine, cellulose, acrylic series resin, etc. by means of chelate, isocyanate, radioactive ray radiation and the like are preferred. Those commercially available include, for example, BR85, BR80, BR113 (manufactured by Mitsubishi Rayon Co., Ltd.) as acrylic resins; APL6509, 130A, 291S, 150R (all manufactured by Mitsui Petrochemical Industries, Ltd.), Zeonex 480, 250, 480S (all manufactured by Nippon Zeon Co., Ltd.) as amorphous polyolefin resins; 3000-1 (manufactured by Denki Kagaku Kogyo K.K.) as polyvinyl butyral resins; SMR-20H, SMR-20HH, C-20, C-10, MA-23, PA-20, PA-15 (all manufactured by Shin-Etsu Chemical Co., Ltd.) as polyvinyl alcohol resins; L-30, Lt-35 (Mitsui Siad Co.) as melamine resins.

In order to improve automatic paper feeding adaptability, at least one of layers constructing the back side of the image-receiving element may comprise an organic and/or inorganic filler. In practice, there are illustrated polyethylene wax, bisamide, nylon, acrylic resin, crosslinked polystyrene, silicone resin, silicone rubber, talc, calcium carbonate, titanium oxide, etc. However, there is no particular limitation and any one can be employed.

Of the above-mentioned, in terms of wear of the paper feeding rubber roller in a printer and decrease in fluctuation of friction characteristics of a roller caused by transport, the nylon filler is particularly preferred. The nylon filler having a molecular weight of 100,000 to 900,000, shape in sphere and average particle diameter of 0.01 to 30  $\mu m$  is preferred and particularly, one having a molecular weight of 100,000 to 500,000 and a average particle diameter of 0.01 to 10  $\mu m$  is more preferred. Further, as the kind of the nylon filler, nylon 12 filler is more preferred than nylon 6 or nylon 66, because the nylon 12 filler is good in water proof and exhibits no change in characteristics by water adsorption.

35

The nylon filler has a high melting point and is thermally stable, bears good oil and chemical resistance and is hardly dyed with dyes. Furthermore, it carries self-lubricating properties and low friction coefficient. When having a molecular weight of 100,000 to 900,000, it is hardly worn and does not damage associate materials. Further, preferred average particle diameter is in the range of from 0.1 to 30  $\mu\text{m}$  in the case of a thermal transfer image receiving element for reflection image and from 0.01 to 1  $\mu\text{m}$  in the case of a thermal transfer image receiving element for transparent image. When the particle diameter is too small, the filler is hidden in the composition layer on the back side and does not achieve fully the slipping function. On the other hand, when the particle diameter is too large, projection from the back side composition layer becomes large to increase the friction coefficient or cause loss of the filler.

Further, any of the above-mentioned fillers are readily available on the market. For example, the polyethylene wax is available as SPRAY30 (manufactured by Sazol Co.) and W950 (Mitsui Petrochemical Industries Ltd.) and as the nylon fillers, for example, MW330 (manufactured by Jinto Toryo Co.) can be illustrated. The added amount of the filler is preferably in the region of from 0.012 to 20 weight parts per 100 weight parts of a binder of the added layer.

The center line average surface roughness Ra on the surface of the back side layer is preferably in the range of from 0.5 to 2.5  $\mu\text{m}$ . In addition, the average number of projections per unit area is preferably from 2,000 to 4,500/ $\text{mm}^2$ . As a method to enable such properties, besides the preparation employing the filler as mentioned above, at the resin extrusion coating, the shape of the surface of the cooling roll is changed to the quality as mentioned above and the formation is performed by transferring the shape when cooling the extruded resin.

In order to increase adhesive force between the back side slipping layer and a base material sheet, an interlayer may be provided between them. As the embodiment of the preferred interlayer, the interlayer having a reaction hardening type resin is provided.

As the reaction hardening type resins, thermosetting resins/ionizing radiation setting resins as described in Japanese Patent Publication Open to Public Inspection No. 6-255276 are preferably employed.

The interlayer having the similar composition may be provided between the basic material sheet and the image-receiving layer.

The image-receiving layer of the present invention may be subjected to treatment to make matte surface and/or to adjust the degree of surface gloss according to the method described in Japanese Patent Publication No. 4-241993.

In the image-receiving element of the present invention, a transparent heat-absorbing substance may be incorporated in the image-receiving layer and/or a layer adjacent to the layer. With the accumulation of heat near the heat absorbing substance, a colorant can be efficiently transferred into the image-receiving layer by expanding it.

As the heat absorbing materials, various kinds of near infrared absorbing dyes are employed. For example, there can be employed nitroso compounds and the metal complexes, polymethine series dyes, squalirium series dyes, thiol nickel salts, phthalocyanine series dyes, triallyl-methane series dyes, naphthoquinone series dyes, anthraquinone series dyes, etc. In addition, many transparent latent heat heat-accumulating materials are employed which are those such as, for example, chain hydrocarbons such as paraffin wax, etc., aromatic hydrocarbons such as paraxylene, etc. phenols, carboxylic acids such as stearic

36

acid, clathrate hydrates such as  $\text{C}_4\text{H}_8\text{O}\cdot117\text{H}_2\text{O}$ , etc., various alcohols, polymeric substances having a low glass transition point such as polyethylene, etc. Furthermore, photochemical reaction utilizing heat accumulating materials utilizing reaction heat generated by light isomerization are employed.

In the image-receiving element, a layer containing air bubbles may be provided to increase cushion property.

As a means of the incorporation of air bubbles, heat expanding hollow particles or capsule-shaped hollow polymers can be utilized. Furthermore, decomposable blowing agents such as dinitropentamethylenetetramine, diaminobenzene, azobisisobutylnitrile, azodicarboamide, etc. may be utilized which are decomposed with heat to generate gases such as oxygen, carbon dioxide, nitrogen, etc.

The kind of the air bubble incorporated in the bubble-containing layer is preferably of dependent air bubbles in terms of the cushion property and heat insulation. For example, those are included which are described in Japanese Patent Publication Open to Public Inspection No. 6-270559.

Furthermore, the air bubble-containing layer itself may incorporate adhesives known in the art. However, in order to increase the adhesion with a base material sheet, a primer layer may be provided between the base material sheet and the air bubble-containing layer. As such the primer layer, for example, those which are described in Japanese Patent Publication Open to Public Inspection No. 5-270152, etc. can be employed.

In the present invention, the image-receiving element and/or the ink sheet may have an antistatic function. In order to enable it to have the antistatic function, conventionally known techniques can be employed. Namely, there can be employed electrically conductive substances such as metals, metal oxides, carbon fine particles, etc., organic compounds termed "antistatic agent" (cation, anion, amphi-ion or non-ion surface active agents or polysiloxans, etc.), electronically conductive inorganic fine particles (fine particles of titanium oxide, zinc oxide, indium oxide, etc. are mixed with impurities and sintered to enhance electronic conductivity disturbing crystal lattice and those which undergo doping treatment, etc.). The electrically conductive substances such as mentioned above may be incorporated into at least one of layers constructing the image-receiving element and/or the ink sheet and at least one layer may be formed as an electrically conductive layer prepared by coating the composition comprising an electrically conductive substance. Naturally, combinations of those are preferably employed.

An electroconductive material is employed for the anti-static layer, coating composition for the electroconductive material is prepared by the usual way. Preferably the anti-static agent is employed in the form of alcohol or aqueous solution, an organic fine powder is used in the form as itself, the former is dissolved or dispersed and the latter is dispersed in the organic solvent composition dissolving resin to form binder.

The resin to form binder is preferably selected from a thermoset resin such as polyacrylic acid ester resin and polyurethane resin, and a thermoplastic resin such as polyvinylchloride resin, polyvinylbutyral resin and polyester resin. Ratio of binder amount to electroconductive material is preferably selected so that the surface resistivity is  $1\times10^{10}$   $\Omega\text{cm}$  or less.

The coating composition of electroconductive material thus prepared is coated by usual coating method such as blade coating, gravure coating or spray coating.

When a static charge processing capability is rendered by providing an electrically conductive layer on a paper

substrate, the aqueous solution of the antistatic agent is preferably coated, or the above-mentioned electronically conductive inorganic fine powders are dispersed or dissolved in aqueous paints such as synthetic resin emulsion, synthetic rubber latex, aqueous solution of a water-soluble resin, etc. and the resulting is preferably coat dried to form the dried layer. As the synthetic resin emulsions, there are exemplified emulsions of polyacrylic acid ester resin or polyurethane resin, etc., and as the synthetic rubber latex, there are exemplified rubber such as methylmethacrylate-butadiene, styrene-butadiene, etc., and as the aqueous solution of the water-soluble resin, aqueous solutions of polyvinyl alcohol resin, polyacrylamide resin, starch, etc. Or more simply, the aqueous solution of an antistatic agent may be spray coated.

Furthermore, as another preferred embodiment, when an antistatic layer is provided on the image-receiving element, or a core material or base material, an antistatic layer composed of the antistatic resins consisting of an acrylic resin and epoxy resin as described in Japanese Patent Publication Open to Public Inspection No. 8-52945.

Such the antistatic layer can be formed by coating a coating solution prepared by mixing the above-mentioned main agent and a hardening agent in a proper ratio on at least one side of the core material or base material of the ink sheet and/or image-receiving element or a primer or adhesive layer provided on those. The antistatic layer is provided on the surface of a core material or base material forming the ink layer or image-receiving layer and on that the ink layer or the image-receiving layer may be provided and may be also provided on the surface of the reverse side of the side on which the ink layer or image-receiving layer is formed. Furthermore, another layer on the side of the antistatic layer, for example, a heat resistant slipping layer or back side slipping layer, etc. may be provided. As the coating method, a conventionally used coating method may be employed.

When the antistatic agent is employed in the image-receiving layer, it is preferably soluble in organic solvent. As the antistatic agents soluble in the organic, those described in Japanese Patent Publication Open to Public Inspection No. 5-64979 are illustrated.

When the above-mentioned antistatic agent is incorporated into the image-receiving layer, the added amount is preferably in the range of 0.1 to 10 parts by weight per 100 parts by weight of the resin forming the image-receiving layer. When the used amount is too little, antistatic effect becomes insufficient, and on the other hand, the excessive amount is not preferred because the dye acceptability of the image-receiving layer and image preservation quality is degraded. In addition, the preferred distribution of the antistatic agent in the direction of the thickness of the image-receiving layer is that 50 weight percent of the antistatic agent is incorporated within  $\frac{1}{3}$  thickness from the surface of the image-receiving layer. When constructed as mentioned above, excellent antistatic property is consistently offered, though dye transfer to the same region of the image-receiving layer is carried out a plurality of times. Further, in order to construct as mentioned above, the image-receiving layer is prepared by slow drying condition and the antistatic agent having a smaller molecular weight than that of a resin is preferably distributed densely at the surface region of the image-receiving layer.

As the post chelate dyes incorporated in the ink layer in the dye-containing region, a dye of which the thermal transfer is possible and various compounds known in the art can be selected and employed. Preferably the dye is sublimable. Specifically, cyan dyes, magenta dyes, yellow dyes,

etc. described in, for example, Japanese Patent Publication Open to Public Inspection Nos. 59-78893, 59-109349, 2-2133032-214719 and 2-203742 can be employed. Of the above-mentioned dyes, dyes which can form two-ligand chelate with the metal source are preferably employed. As such dyes, for example, those represented by the general formula (2) described below can be illustrated.



General formula (2)

In the above-mentioned general formula (2),  $X_1$  represents a group of atoms necessary to complete an aromatic carbon ring or heterocyclic ring in which at least one of rings is composed of 5 to 7 atoms and at least one of positions adjacent to the carbon atom joined with an azo bond is a nitrogen atom or a carbon atom replaced with a chelated group.  $X_2$  represents an aromatic heterocyclic ring or aromatic carbon ring in which at least one of rings is composed of 5 to 7 atoms. G represents a chelated group. The used amount of the above-mentioned dye is generally in the range of from 0.1 to 20 g per 1 m<sup>2</sup> of an ink sheet and preferably from 0.2 to 5 g.

The ratio by weight of a binder to a dye is preferably in the range of from 1:10 to 10:1 and more preferably in the range of from 2:8 to 7:3.

On the ink sheet, various kinds of additives other than the above-mentioned compounds can be suitably added. As the additives, as mentioned above, there are illustrated lubricating compounds such as silicone resins, silicone oils (reaction hardening type available), silicone modified resins, fluoro resins, surface active agents and waxes, fillers such as metal powder, silica gel, metal oxides, carbon black, resin fine particles, etc., hardening agents (for example, radiation active compounds such as isocyanates, acrylic compounds, epoxy compounds) capable of reacting with a binder constituent, etc.

The ink sheet includes the two-layer construction consisting of a support and an ink layer and also the other layer may be formed thereon. For example, with the object of preventing melt-adhesion with the image-receiving layer and dye transfer to a back side (blocking), an overcoat layer may be provided on the surface of the above-mentioned ink layer.

Furthermore, in order to improve the adhesion with the binder of an ink layer and prevent the transfer of a sublimable dye to the side of the support and dying caused by it, the support having thereon an ink sheet may have thereon a subbing layer. Further, on the back side (reverse side of the ink layer) of the support, a sticking prevention layer may be provided in order to prevent the melt-adhesion or sticking of a head to the support and the formation of wrinkles in the ink sheet. Each of the thickness of the above-mentioned overcoat layer, subbing layer and sticking prevention layer is from 0.1 to 1  $\mu$ m.

## EXAMPLE

The present invention is specifically explained with reference to Examples. Moreover, "parts" in Example are "by weight".

### Example 1 Preparation of Ink Sheet 1

Each ink layer composed of the following composition of yellow, magenta cyan were coated (coating amount of 1.1 g/m<sup>2</sup> after drying) on the back side of a heat resistant protective layer (SP-712, product of Dainichiseika, Co, Ltd.) of polyethylene terephthalate film (Rumilar 6CF531 manu-

factured by Toray Industries, Inc.) having a thickness of 6  $\mu\text{m}$  and the above-mentioned protective layer by a gravure method, and the ink sheet was prepared in which each ink layer of yellow, magenta and cyan, and the metal source-containing layer are arranged in order (hereinafter referred to as "face order") as shown in FIG. 1.

| <u>Yellow Ink Layer</u>              |           |
|--------------------------------------|-----------|
| Post chelate dye Y-1 mentioned below | 3 parts   |
| Polyvinyl acetal (Denkabutyril       | 5.5 parts |
| KY-24 manufactured by Denki Kagaku   |           |
| Kogyo K.K.)                          |           |
| Polymethylmethacrylate (Rezeda       | 1 parts   |
| GP-305 manufactured by Toagosei      |           |
| Co., Ltd.)                           |           |
| Urethane modified silicone oil       | 0.5 parts |
| (Diaroma SP-2105 manufactured by     |           |
| Dainichiseika Color & Chemicals      |           |
| Mfg. Co., Ltd.)                      |           |
| Methylethylketone                    | 80 parts  |
| Toluene                              | 10 parts  |
| <u>Magenta Ink Layer</u>             |           |
| Post chelate dye M-1 mentioned below | 3 parts   |
| Polyvinyl acetal (Denkabutyril       | 5.5 parts |
| KY-24 manufactured by Denki Kagaku   |           |
| Kogyo K.K.)                          |           |
| Polymethylmethacrylate (Rezeda       | 1 parts   |
| GP-305 manufactured by Toagosei      |           |
| Co., Ltd.)                           |           |
| Urethane modified silicone oil       | 0.5 parts |
| (Diaroma SP-2105 manufactured by     |           |
| Dainichiseika Color & Chemicals      |           |
| Mfg. Co., Ltd.)                      |           |
| Methylethylketone                    | 80 parts  |
| Toluene                              | 10 parts  |
| <u>Cyan Ink Layer</u>                |           |
| Post chelate dye C-1 mentioned below | 3 parts   |
| Polyvinyl acetal (Denkabutyril       | 5.5 parts |
| KY-24 manufactured by Denki Kagaku   |           |
| Kogyo K.K.)                          |           |
| Polymethylmethacrylate (Rezeda       | 1 parts   |
| GP-305 manufactured by Toagosei      |           |
| Co., Ltd.)                           |           |
| Urethane modified silicone oil       | 0.5 parts |
| (Diaroma SP-2105 manufactured by     |           |
| Dainichiseika Color & Chemicals      |           |
| Mfg. Co., Ltd.)                      |           |
| Methylethylketone                    | 80 parts  |
| Toluene                              | 10 parts  |
| <u>Re-heating layer</u>              |           |
| Polyvinyl acetal (Denkabutyril       | 6 parts   |
| KY-24 manufactured by Denki Kagaku   |           |
| Kogyo K.K.)                          |           |
| Polymethylmethacrylate (Rezeda       | 2 parts   |
| GP-305 manufactured by Toagosei      |           |
| Co., Ltd.)                           |           |
| Urethane modified silicone oil       | 2 parts   |
| (Diaroma SP-2105 manufactured by     |           |
| Dainichiseika Color & Chemicals      |           |
| Mfg. Co., Ltd.)                      |           |
| Methylethylketone                    | 80 parts  |
| Toluene                              | 10 parts  |

Y-1



M-1



C-1



#### Preparation of Image-receiving Sheet 1

On the surface of a synthetic paper having thickness of 118  $\mu\text{m}$  (Lumilar E60L manufactured by Toray Co., Ltd.), an anchor layer and image-receiving layer, each of composition is shown below, were coated in this order, so as to result in thickness of 2  $\mu\text{m}$ , and 4  $\mu\text{m}$ , respectively and thus the image-receiving sheet was prepared.

35

#### Anchor Layer

|                                                                   |           |
|-------------------------------------------------------------------|-----------|
| Polyvinyl acetoacetal                                             | 7.5 Parts |
| (Eslex BL-1 manufactured by Sekisui Chemical Co., Ltd.)           |           |
| Isocyanate                                                        | 2.5 parts |
| (Coronate HX manufactured by Nippon Polyurethane Kogyo Co., Ltd.) |           |
| Methylethylketone                                                 | 80 parts  |
| n-Butylacetate                                                    | 10 parts  |
| <u>Image-receiving Layer</u>                                      |           |

|                                                          |           |
|----------------------------------------------------------|-----------|
| Polyvinyl butyral                                        | 9.5 parts |
| (Eslex BX-1 manufactured by Sekisui Chemical Co., Ltd.)  |           |
| Polyester modified silicone                              | 0.5 part  |
| (X-24-8300 manufactured by Shin-Etsu Chemical Co., Ltd.) |           |
| Methylethylketone                                        | 80 parts  |
| n-Butylacetate                                           | 10 parts  |

#### Image Formation

55 The image receiving part of the image receiving sheet and the ink layer part of the ink sheet thus prepared were brought into contact, then they were pressed by a thermal head having image definition of 12 dot/mm and average resistance of 3100 ohm and platen roll, they were heated from the 60 back side of ink layer with power supplying period of 10 msec/line in accordance with signals of step pattern of increasing supplying energy from 5 to 80 mJ/mm<sup>2</sup> for yellow, magenta, cyan and neutral (combination of yellow, magenta and cyan) image to transfer the dyes to the image receiving sheet. Then, pressing the re-heat layer and superposed image transferred image receiving sheet by the same thermal head and the same platen roll, they were heated from 65

the back side of the re-heating layer with the condition of supplying energy and power supplying period shown in Table 1.

No blurring or omission of image was not found in the obtained image by employing each sheet with the above mentioned process.

The following evaluation were carried out for the obtained image of the Sample 1 to 40.

#### Evaluation on Surface Characteristics

The change of the surface condition before and after the re-heating process was visually evaluated. The glossiness of the surface will reduce to become matting surface by heating. In case that image is not formed on the whole image receiving sheet, boundary of the image area and non-image area appears to reduce the image quality. Standard of the evaluation are as follows;

A: No boundary appears.

B: Boundary appears depending on viewing angle, but no problem in practical viewing.

C: Marked boundary appears unsightly.

#### Evaluation on Uneven Band Image

Uneven band found in image caused by the transporting system was observed at the maximum density area of neutral image. Standard of the evaluation are as follows;

4: No uneven band is observed.

3: Uneven band is observed depending on viewing angle, but no problem in practical viewing.

2: Uneven band is observed at a glance.

1: Marked uneven band is observed unsightly.

#### Evaluation on Light Fastness of Images

Each of the above-mentioned images around the area at dye image density of 1.0 was subjected to exposure by a xenon fade-o-meter (70,000 lux) for 14 days and each density was measured to obtain a density remaining ratio. The higher chelation ratio after re-heating process is obtained, the higher density remaining ratio is given. It is preferable that the density remaining ratio is not less than 70%.

Image density was measured by X-Rite 310TR, manufactured by X-Rite Corporation.

#### Evaluation on Transportation

Image formation of 100 sheets with each control condition were carried out, wherein number of sticking occurrence were counted.

#### Preservation Evaluation Stored in Album

The image having neutral patch of visual density of  $1.5 \pm 0.1$  prepared above was interposed between album paper and transparent cover sheet (A-194N, manufactured by Kokuyo Co., LTD.) and stored for 28 days under condition of pressure of  $20 \text{ g/cm}^2$ , at  $50^\circ \text{C}$ , and 80% RH. Image density transferred to the transparent cover sheet was measured. Image density was measured by the same apparatus as that employed for the evaluation of light fastness. The transferred image density is preferably 0.3 or less.

The result is summarized in Tables 2 and 3.

TABLE 2

| Sam-<br>ple | Ink<br>sheet | Image<br>receiving<br>sheet | Applied<br>energy | Power<br>supplying<br>period | Surface<br>condi-<br>tion | Image | Light stability |     |                    | Album<br>preser-<br>vation | Number<br>of<br>sticking |
|-------------|--------------|-----------------------------|-------------------|------------------------------|---------------------------|-------|-----------------|-----|--------------------|----------------------------|--------------------------|
|             |              |                             |                   |                              |                           |       | No.             | No. | mJ/mm <sup>2</sup> | msec/line                  |                          |
| 1**         | 1            | 1                           | —                 | —                            | A                         | 4     | 68              | 67  | 60                 | 0.085                      | 0                        |
| 2           | 1            | 1                           | 80                | 100 %                        | B                         | 2     | 79              | 80  | 74                 | 0.027                      | 3                        |
| 3           | 1            | 1                           | 80                | 100                          | C                         | 2     | 85              | 84  | 85                 | 0.016                      | 5                        |
| 4           | 1            | 1                           | 80                | 100                          | C                         | 1     | 87              | 86  | 86                 | 0.005                      | 7                        |
| 5           | 1            | 1                           | 80                | 100                          | C                         | 1     | *               | *   | *                  | *                          | *                        |
| 6           | 1            | 1                           | 80                | 100                          | C                         | 1     | *               | *   | *                  | *                          | *                        |
| 7           | 1            | 1                           | 68                | 85                           | B                         | 3     | 77              | 77  | 68                 | 0.035                      | 0                        |
| 8           | 1            | 1                           | 68                | 85                           | B                         | 3     | 81              | 81  | 79                 | 0.024                      | 0                        |
| 9           | 1            | 1                           | 68                | 85                           | B                         | 3     | 83              | 83  | 85                 | 0.019                      | 0                        |
| 10          | 1            | 1                           | 68                | 85                           | B                         | 3     | 84              | 84  | 87                 | 0.014                      | 0                        |
| 11          | 1            | 1                           | 68                | 85                           | B                         | 3     | 85              | 85  | 88                 | 0.014                      | 0                        |
| 12          | 1            | 1                           | 60                | 75                           | A                         | 4     | 74              | 74  | 66                 | 0.041                      | 0                        |
| 13          | 1            | 1                           | 60                | 75                           | B                         | 4     | 78              | 80  | 76                 | 0.027                      | 0                        |
| 14          | 1            | 1                           | 60                | 75                           | B                         | 4     | 81              | 81  | 83                 | 0.024                      | 0                        |
| 15          | 1            | 1                           | 60                | 75                           | B                         | 4     | 83              | 82  | 86                 | 0.019                      | 0                        |
| 16          | 1            | 1                           | 60                | 75                           | B                         | 3     | 84              | 83  | 86                 | 0.014                      | 0                        |
| 17          | 1            | 1                           | 60                | 75                           | B                         | 3     | 85              | 83  | 86                 | 0.014                      | 0                        |
| 18          | 1            | 1                           | 50                | 63                           | A                         | 4     | 71              | 71  | 64                 | 0.049                      | 0                        |
| 19          | 1            | 1                           | 50                | 63                           | A                         | 4     | 76              | 77  | 74                 | 0.027                      | 0                        |
| 20          | 1            | 1                           | 50                | 63                           | A                         | 4     | 78              | 79  | 81                 | 0.024                      | 0                        |

\*Image receiving layer and re-heating layer are fused and evaluation was not possible.

\*\*No re-heating was applied.

TABLE 3

| Sam-<br>ple | Ink<br>sheet | Image<br>receiving<br>sheet | Applied<br>energy | Power<br>supplying<br>period | Surface<br>condi-<br>tion | Image | Light stability |     |                    | Album<br>preser-<br>vation | Number<br>of<br>sticking |   |
|-------------|--------------|-----------------------------|-------------------|------------------------------|---------------------------|-------|-----------------|-----|--------------------|----------------------------|--------------------------|---|
|             |              |                             |                   |                              |                           |       | No.             | No. | mJ/mm <sup>2</sup> | msec/line                  |                          |   |
| 21          | 1            | 1                           | 50                | 63 %                         | 7.6                       | 76    | 4               | 82  | 82                 | 85                         | 0.019                    | 0 |
| 22          | 1            | 1                           | 50                | 63                           | 6.6                       | 66    | 4               | 83  | 84                 | 86                         | 0.014                    | 0 |

TABLE 3-continued

| Sam-<br>ple | Ink<br>sheet | Image<br>receiving<br>sheet | Applied<br>energy | Power<br>supplying<br>period | Surface<br>condi-<br>tion | Image | Light stability |        |         | Album<br>preser-<br>vation | Number<br>of<br>sticking |       |   |
|-------------|--------------|-----------------------------|-------------------|------------------------------|---------------------------|-------|-----------------|--------|---------|----------------------------|--------------------------|-------|---|
|             |              |                             |                   |                              |                           |       | unevenness      | Yellow | Magenta | Cyan                       |                          |       |   |
| 23          | 1            | 1                           | 50                | 63                           | 5.6                       | 56    | B               | 3      | 84      | 84                         | 86                       | 0.014 | 0 |
| 24          | 1            | 1                           | 50                | 63                           | 10                        | 100   | A               | 4      | 74      | 75                         | 68                       | 0.027 | 0 |
| 25          | 1            | 1                           | 50                | 63                           | 9.6                       | 96    | A               | 4      | 78      | 79                         | 79                       | 0.014 | 0 |
| 26          | 1            | 1                           | 50                | 63                           | 8.6                       | 86    | A               | 4      | 81      | 81                         | 85                       | 0.011 | 0 |
| 27          | 1            | 1                           | 50                | 63                           | 7.6                       | 76    | A               | 4      | 85      | 85                         | 86                       | 0.005 | 0 |
| 28          | 1            | 1                           | 50                | 63                           | 6.6                       | 66    | A               | 4      | 86      | 86                         | 88                       | 0.005 | 0 |
| 29          | 1            | 1                           | 50                | 63                           | 5.6                       | 56    | B               | 3      | 86      | 86                         | 88                       | 0.005 | 0 |
| 30          | 1            | 1                           | 40                | 50                           | 10                        | 100   | A               | 4      | 69      | 68                         | 62                       | 0.054 | 0 |
| 31          | 1            | 1                           | 40                | 50                           | 9.6                       | 96    | A               | 4      | 74      | 74                         | 72                       | 0.035 | 0 |
| 32          | 1            | 1                           | 40                | 50                           | 8.6                       | 86    | A               | 4      | 78      | 77                         | 78                       | 0.030 | 0 |
| 33          | 1            | 1                           | 40                | 50                           | 7.6                       | 76    | A               | 4      | 81      | 80                         | 82                       | 0.022 | 0 |
| 34          | 1            | 1                           | 40                | 50                           | 6.6                       | 66    | A               | 4      | 82      | 80                         | 84                       | 0.016 | 0 |
| 35          | 1            | 1                           | 40                | 50                           | 5.6                       | 56    | A               | 3      | 82      | 80                         | 85                       | 0.016 | 0 |
| 36          | 1            | 1                           | 30                | 38                           | 10                        | 100   | A               | 4      | 67      | 66                         | 59                       | 0.062 | 0 |
| 37          | 1            | 1                           | 30                | 38                           | 9.6                       | 96    | A               | 4      | 72      | 71                         | 69                       | 0.038 | 0 |
| 38          | 1            | 1                           | 30                | 38                           | 8.6                       | 86    | A               | 4      | 76      | 75                         | 75                       | 0.027 | 0 |
| 39          | 1            | 1                           | 30                | 38                           | 7.6                       | 76    | A               | 4      | 78      | 79                         | 79                       | 0.022 | 0 |
| 40          | 1            | 1                           | 30                | 38                           | 6.6                       | 66    | A               | 4      | 79      | 80                         | 82                       | 0.019 | 0 |

## Example 2

25

-continued

C-2

## Preparation of Ink Sheet 2

Ink Sheet 2 was prepared in the same way as in Ink Sheet 1 except that the dyes employed in each layer of yellow, magenta and cyan were modified by following Y-2, M-2 and C-2 respectively. These are all reactive dyes.

35



Y-2 40

## Preparation of Image Receiving Layer 2

Image Receiving Layer 2 was prepared in the same way as in Image Receiving Layer 1 except that the component was modified as shown below.

45

|    |                                                                                            |           |
|----|--------------------------------------------------------------------------------------------|-----------|
| 50 | Polyvinyl butyral<br>(Eslex BX-1 manufactured by Sekisui<br>Chemical Co., Ltd.)            | 7.9 parts |
|    | Epomine (manufactured by Nippon Shokubai Co., Ltd.)                                        | 1.6 parts |
|    | Polyester modified silicone<br>(X-24-8300 manufactured by<br>Shin-Etsu Chemical Co., Ltd.) | 0.5 part  |
| 55 | Methyl ethyl ketone                                                                        | 80 parts  |
|    | Toluene                                                                                    | 10 parts  |



## 60 Image Formation and Evaluation

Image was formed and evaluated for the Samples 41 to 80 in the same way as Example 1. The result is summarized in Tables 4 and 5.

65

TABLE 4

| Sam-<br>ple | Ink<br>sheet | Image<br>receiving<br>sheet | Applied<br>energy | Power<br>supplying<br>period | Surface<br>condi-<br>tion | Image | Light stability    |           |            | Album<br>preser-<br>vation | Number<br>of<br>sticking |      |
|-------------|--------------|-----------------------------|-------------------|------------------------------|---------------------------|-------|--------------------|-----------|------------|----------------------------|--------------------------|------|
|             |              |                             |                   |                              |                           |       | mJ/mm <sup>2</sup> | msec/line | unevenness | Yellow                     | Magenta                  | Cyan |
| 41**        | 2            | 2                           | —                 | —                            | —                         | A     | 4                  | 66        | 66         | 57                         | 0.072                    | 0    |
| 42          | 2            | 2                           | 80                | 100                          | %                         | B     | 2                  | 81        | 83         | 74                         | 0.022                    | 3    |
| 43          | 2            | 2                           | 80                | 100                          |                           | C     | 2                  | 87        | 87         | 85                         | 0.013                    | 5    |
| 44          | 2            | 2                           | 80                | 100                          |                           | C     | 1                  | 89        | 89         | 86                         | 0.004                    | 7    |
| 45          | 2            | 2                           | 80                | 100                          |                           | C     | 1                  | *         | *          | *                          | *                        | *    |
| 46          | 2            | 2                           | 80                | 100                          |                           | C     | 1                  | *         | *          | *                          | *                        | *    |
| 47          | 2            | 2                           | 68                | 85                           |                           | B     | 3                  | 78        | 80         | 68                         | 0.028                    | 0    |
| 48          | 2            | 2                           | 68                | 85                           |                           | B     | 3                  | 83        | 84         | 79                         | 0.020                    | 0    |
| 49          | 2            | 2                           | 68                | 85                           |                           | B     | 3                  | 85        | 86         | 85                         | 0.015                    | 0    |
| 50          | 2            | 2                           | 68                | 85                           |                           | B     | 3                  | 86        | 87         | 87                         | 0.011                    | 0    |
| 51          | 2            | 2                           | 68                | 85                           |                           | B     | 3                  | 87        | 88         | 88                         | 0.011                    | 0    |
| 52          | 2            | 2                           | 60                | 75                           |                           | A     | 4                  | 75        | 77         | 66                         | 0.033                    | 0    |
| 53          | 2            | 2                           | 60                | 75                           |                           | B     | 4                  | 80        | 83         | 76                         | 0.022                    | 0    |
| 54          | 2            | 2                           | 60                | 75                           |                           | B     | 4                  | 83        | 84         | 83                         | 0.020                    | 0    |
| 55          | 2            | 2                           | 60                | 75                           |                           | B     | 4                  | 85        | 85         | 86                         | 0.015                    | 0    |
| 56          | 2            | 2                           | 60                | 75                           |                           | B     | 3                  | 86        | 86         | 86                         | 0.011                    | 0    |
| 57          | 2            | 2                           | 60                | 75                           |                           | B     | 3                  | 87        | 86         | 86                         | 0.011                    | 0    |
| 58          | 2            | 2                           | 50                | 63                           |                           | A     | 4                  | 73        | 74         | 64                         | 0.039                    | 0    |
| 59          | 2            | 2                           | 50                | 63                           |                           | A     | 4                  | 77        | 80         | 74                         | 0.022                    | 0    |
| 60          | 2            | 2                           | 50                | 63                           |                           | A     | 4                  | 80        | 82         | 81                         | 0.020                    | 0    |

\*Image receiving layer and re-heating layer are fused and evaluation was not possible.

\*\*No re-heating was applied.

TABLE 5

| Sam-<br>ple | Ink<br>sheet | Image<br>receiving<br>sheet | Applied<br>energy | Power<br>supplying<br>period | Surface<br>condi-<br>tion | Image | Light stability    |           |            | Album<br>preser-<br>vation | Number<br>of<br>sticking |      |
|-------------|--------------|-----------------------------|-------------------|------------------------------|---------------------------|-------|--------------------|-----------|------------|----------------------------|--------------------------|------|
|             |              |                             |                   |                              |                           |       | mJ/mm <sup>2</sup> | msec/line | unevenness | Yellow                     | Magenta                  | Cyan |
| 61          | 2            | 2                           | 50                | 63                           | %                         | A     | 4                  | 84        | 85         | 85                         | 0.015                    | 0    |
| 62          | 2            | 2                           | 50                | 63                           |                           | A     | 4                  | 85        | 87         | 86                         | 0.011                    | 0    |
| 63          | 2            | 2                           | 50                | 63                           |                           | B     | 3                  | 86        | 87         | 86                         | 0.011                    | 0    |
| 64          | 2            | 2                           | 50                | 63                           |                           | A     | 4                  | 75        | 78         | 68                         | 0.022                    | 0    |
| 65          | 2            | 2                           | 50                | 63                           |                           | A     | 4                  | 80        | 82         | 79                         | 0.011                    | 0    |
| 66          | 2            | 2                           | 50                | 63                           |                           | A     | 4                  | 83        | 84         | 85                         | 0.009                    | 0    |
| 67          | 2            | 2                           | 50                | 63                           |                           | A     | 4                  | 87        | 88         | 86                         | 0.004                    | 0    |
| 68          | 2            | 2                           | 50                | 63                           |                           | A     | 4                  | 88        | 89         | 88                         | 0.004                    | 0    |
| 69          | 2            | 2                           | 50                | 63                           |                           | B     | 3                  | 88        | 89         | 88                         | 0.004                    | 0    |
| 70          | 2            | 2                           | 40                | 50                           |                           | A     | 4                  | 71        | 71         | 62                         | 0.044                    | 0    |
| 71          | 2            | 2                           | 40                | 50                           |                           | A     | 4                  | 75        | 77         | 72                         | 0.028                    | 0    |
| 72          | 2            | 2                           | 40                | 50                           |                           | A     | 4                  | 79        | 80         | 78                         | 0.024                    | 0    |
| 73          | 2            | 2                           | 40                | 50                           |                           | A     | 4                  | 83        | 83         | 82                         | 0.017                    | 0    |
| 74          | 2            | 2                           | 40                | 50                           |                           | A     | 4                  | 84        | 83         | 84                         | 0.013                    | 0    |
| 75          | 2            | 2                           | 40                | 50                           |                           | A     | 3                  | 84        | 83         | 85                         | 0.013                    | 0    |
| 76          | 2            | 2                           | 30                | 38                           |                           | A     | 4                  | 69        | 68         | 59                         | 0.050                    | 0    |
| 77          | 2            | 2                           | 30                | 38                           |                           | A     | 4                  | 74        | 74         | 69                         | 0.031                    | 0    |
| 78          | 2            | 2                           | 30                | 38                           |                           | A     | 4                  | 77        | 78         | 75                         | 0.022                    | 0    |
| 79          | 2            | 2                           | 30                | 38                           |                           | A     | 4                  | 79        | 82         | 79                         | 0.017                    | 0    |
| 80          | 2            | 2                           | 30                | 38                           |                           | A     | 4                  | 81        | 83         | 82                         | 0.015                    | 0    |

## Example 3

## Preparation of Ink Sheet 3

Ink Sheet 3 was prepared in the same way as in Ink Sheet 1 except that the dyes employed in each layer of yellow, magenta and cyan were replaced by those shown below.

Yellow dye: Exemplified compound (26)

Magenta dye: Exemplified compound (25)

Cyan dye: Exemplified compound (28)

## Preparation of Ink Sheet 4

Ink Sheet 4 was prepared in the same way as in Example 1 except that the Re-heating layer was modified by the following composition.

## Re-heating layer

|                                                                                                    |           |
|----------------------------------------------------------------------------------------------------|-----------|
| (Metal Source (MS-1))                                                                              | 0.1 part  |
| $\text{Ni}^{2+} (\text{NH}_2\text{COCH}_2\text{NH}_2)_3 \cdot 2\text{B}(\text{C}_6\text{H}_5)_4^-$ | 5.9 parts |
| Polyvinyl acetal (KY-24 manufactured by Denki Kagaku Kogyo K.K.)                                   |           |
| Polymethylmethacrylate (Rezeda GP-305 manufactured by Toagosei Co., Ltd.)                          | 2 parts   |
| Urethane modified silicone oil (Diaroma SP-2105 manufactured by Dainichiseika Color & Chemicals    | 2 parts   |

-continued

|                   |                                     |           |
|-------------------|-------------------------------------|-----------|
| Mfg. Co., Ltd.)   | Polyvinyl butyral                   | 6.5 parts |
| Methylethylketone | (Eslex BX-1 manufactured by Sekisui |           |
| Toluene           | Chemical Co., Ltd.)                 |           |
|                   | Metal source 1 (MS-1)               | 3 parts   |
|                   | Polyester modified silicone         | 0.5 part  |
|                   | (X-24-8300 manufactured by          |           |
|                   | Shin-Etsu Chemical Co., Ltd.)       |           |
|                   | Methylethylketone                   | 80 parts  |
| 5                 | n-Butylacetate                      | 10 parts  |

## Preparation of Image Receiving Sheet 3

Image Receiving Sheet 4 was prepared in the same way as in Example 1 except that the Re-heating layer was modified by the following composition.

## Image Formation and Evaluation

Image was formed and evaluated for the Samples 81 to 120 in the same way as Example 1. The result is summarized in Tables 6 and 7.

TABLE 6

| Sam-<br>ple | Ink<br>sheet | Image<br>receiving<br>sheet | Applied<br>energy  | Power<br>supplying<br>period | Surface<br>condi-<br>tion | Image | Light stability |        |         | Album<br>preser-<br>vation | Number<br>of<br>sticking |       |   |
|-------------|--------------|-----------------------------|--------------------|------------------------------|---------------------------|-------|-----------------|--------|---------|----------------------------|--------------------------|-------|---|
|             |              |                             |                    |                              |                           |       | unevenness      | Yellow | Magenta |                            |                          |       |   |
| No.         | No.          | No.                         | mJ/mm <sup>2</sup> | msec/line                    |                           |       |                 |        |         |                            |                          |       |   |
| 81**        | 3            | 3                           | —                  | —                            | —                         | A     | 4               | 70     | 68      | 58                         | 0.033                    | 0     |   |
| 82          | 3            | 3                           | 80                 | 100                          | %                         | B     | 2               | 86     | 85      | 75                         | 0.01                     | 3     |   |
| 83          | 3            | 3                           | 80                 | 100                          |                           | C     | 2               | 92     | 90      | 86                         | 0.006                    | 5     |   |
| 84          | 3            | 3                           | 80                 | 100                          |                           | C     | 1               | 94     | 92      | 88                         | 0.002                    | 7     |   |
| 85          | 3            | 3                           | 80                 | 100                          |                           | C     | 1               | *      | *       | *                          | *                        | *     |   |
| 86          | 3            | 3                           | 80                 | 100                          |                           | C     | 1               | *      | *       | *                          | *                        | *     |   |
| 87          | 3            | 3                           | 68                 | 85                           | 10                        | 100   | B               | 3      | 83      | 82                         | 69                       | 0.013 | 0 |
| 88          | 3            | 3                           | 68                 | 85                           | 9.6                       | 96    | B               | 3      | 88      | 87                         | 80                       | 0.009 | 0 |
| 89          | 3            | 3                           | 68                 | 85                           | 8.6                       | 86    | B               | 3      | 90      | 89                         | 86                       | 0.007 | 0 |
| 90          | 3            | 3                           | 68                 | 85                           | 7.6                       | 76    | B               | 3      | 91      | 90                         | 89                       | 0.005 | 0 |
| 91          | 3            | 3                           | 68                 | 85                           | 6.6                       | 66    | B               | 3      | 92      | 91                         | 90                       | 0.005 | 0 |
| 92          | 3            | 3                           | 60                 | 75                           | 10                        | 100   | A               | 4      | 80      | 79                         | 67                       | 0.015 | 0 |
| 93          | 3            | 3                           | 60                 | 75                           | 9.6                       | 96    | B               | 4      | 85      | 85                         | 77                       | 0.01  | 0 |
| 94          | 3            | 3                           | 60                 | 75                           | 8.6                       | 86    | B               | 4      | 88      | 87                         | 84                       | 0.009 | 0 |
| 95          | 3            | 3                           | 60                 | 75                           | 7.6                       | 76    | B               | 4      | 90      | 88                         | 87                       | 0.007 | 0 |
| 96          | 3            | 3                           | 60                 | 75                           | 6.6                       | 66    | B               | 3      | 91      | 89                         | 88                       | 0.005 | 0 |
| 97          | 3            | 3                           | 60                 | 75                           | 5.6                       | 56    | B               | 3      | 92      | 89                         | 88                       | 0.005 | 0 |
| 98          | 3            | 3                           | 50                 | 63                           | 10                        | 100   | A               | 4      | 77      | 76                         | 65                       | 0.018 | 0 |
| 99          | 3            | 3                           | 50                 | 63                           | 9.6                       | 96    | A               | 4      | 82      | 82                         | 75                       | 0.01  | 0 |
| 100         | 3            | 3                           | 50                 | 63                           | 8.6                       | 86    | A               | 4      | 85      | 84                         | 82                       | 0.009 | 0 |

\*Image receiving layer and re-heating layer are fused and evaluation was not possible.

\*\*No re-heating was applied.

TABLE 7

| Sam-<br>ple | Ink<br>sheet | Image<br>receiving<br>sheet | Applied<br>energy  | Power<br>supplying<br>period | Surface<br>condi-<br>tion | Image | Light stability |        |         | Album<br>preser-<br>vation | Number<br>of<br>sticking |    |    |       |   |
|-------------|--------------|-----------------------------|--------------------|------------------------------|---------------------------|-------|-----------------|--------|---------|----------------------------|--------------------------|----|----|-------|---|
|             |              |                             |                    |                              |                           |       | unevenness      | Yellow | Magenta |                            |                          |    |    |       |   |
| No.         | No.          | No.                         | mJ/mm <sup>2</sup> | msec/line                    |                           |       |                 |        |         |                            |                          |    |    |       |   |
| 101         | 3            | 3                           | 50                 | 63                           | %                         | 7.6   | 76              | %      | A       | 4                          | 89                       | 88 | 86 | 0.007 | 0 |
| 102         | 3            | 3                           | 50                 | 63                           |                           | 6.6   | 66              |        | A       | 4                          | 90                       | 90 | 87 | 0.005 | 0 |
| 103         | 3            | 3                           | 50                 | 63                           |                           | 5.6   | 56              |        | B       | 3                          | 91                       | 90 | 88 | 0.005 | 0 |
| 104         | 4            | 3                           | 50                 | 63                           |                           | 10    | 100             |        | A       | 4                          | 80                       | 80 | 69 | 0.01  | 0 |
| 105         | 4            | 3                           | 50                 | 63                           |                           | 9.6   | 96              |        | A       | 4                          | 85                       | 84 | 80 | 0.005 | 0 |
| 106         | 4            | 3                           | 50                 | 63                           |                           | 8.6   | 86              |        | A       | 4                          | 88                       | 87 | 86 | 0.004 | 0 |
| 107         | 4            | 3                           | 50                 | 63                           |                           | 7.6   | 76              |        | A       | 4                          | 92                       | 91 | 88 | 0.002 | 0 |
| 108         | 4            | 3                           | 50                 | 63                           |                           | 6.6   | 66              |        | A       | 4                          | 93                       | 92 | 90 | 0.002 | 0 |
| 109         | 4            | 3                           | 50                 | 63                           |                           | 5.6   | 56              |        | B       | 3                          | 93                       | 92 | 90 | 0.002 | 0 |
| 110         | 3            | 3                           | 40                 | 50                           |                           | 10    | 100             |        | A       | 4                          | 75                       | 73 | 63 | 0.02  | 0 |
| 111         | 3            | 3                           | 40                 | 50                           |                           | 9.6   | 96              |        | A       | 4                          | 80                       | 79 | 73 | 0.013 | 0 |
| 112         | 3            | 3                           | 40                 | 50                           |                           | 8.6   | 86              |        | A       | 4                          | 84                       | 82 | 79 | 0.011 | 0 |
| 113         | 3            | 3                           | 40                 | 50                           |                           | 7.6   | 76              |        | A       | 4                          | 88                       | 85 | 83 | 0.008 | 0 |
| 114         | 3            | 3                           | 40                 | 50                           |                           | 6.6   | 66              |        | A       | 4                          | 89                       | 86 | 85 | 0.006 | 0 |
| 115         | 3            | 3                           | 40                 | 50                           |                           | 5.6   | 56              |        | A       | 3                          | 89                       | 86 | 86 | 0.006 | 0 |
| 116         | 3            | 3                           | 30                 | 38                           |                           | 10    | 100             |        | A       | 4                          | 73                       | 70 | 60 | 0.023 | 0 |
| 117         | 3            | 3                           | 30                 | 38                           |                           | 9.6   | 96              |        | A       | 4                          | 78                       | 76 | 70 | 0.014 | 0 |
| 118         | 3            | 3                           | 30                 | 38                           |                           | 8.6   | 86              |        | A       | 4                          | 82                       | 80 | 76 | 0.01  | 0 |
| 119         | 3            | 3                           | 30                 | 38                           |                           | 7.6   | 76              |        | A       | 4                          | 84                       | 84 | 80 | 0.008 | 0 |
| 120         | 3            | 3                           | 30                 | 38                           |                           | 6.6   | 66              |        | A       | 4                          | 86                       | 83 | 83 | 0.007 | 0 |

## Example 4

## Preparation of Ink Sheet 5

Ink Sheet 5 was prepared in the way that monochrome ink layer was formed in place of yellow, magenta and cyan ink layer of Example 1. In the Ink sheet 5 monochrome ink area and re-heating area were placed alternatively.

-continued

|    |                                                                                                                                                              |                                  |           |
|----|--------------------------------------------------------------------------------------------------------------------------------------------------------------|----------------------------------|-----------|
| 5  | Co., Ltd.)                                                                                                                                                   | Urethane modified silicone oil   | 0.5 parts |
|    | Dainichiseika Color & Chemicals                                                                                                                              | (Diaroma SP-2105 manufactured by |           |
|    | Mfg. Co., Ltd.)                                                                                                                                              | Dainichiseika Color & Chemicals  |           |
|    | Methylethylketone                                                                                                                                            |                                  | 80 parts  |
|    | Toluene                                                                                                                                                      |                                  | 10 parts  |
| 10 |                                                                                                                                                              |                                  |           |
|    | Image Formation                                                                                                                                              |                                  |           |
|    | Monochrome image was formed in the same way as Example 1 by employing the Image Receiving Sheet 3.                                                           |                                  |           |
| 15 | Samples 121–160 were evaluated in the same as Example 1. Light fastness was measured by means of visual density. The result is summarized in Tables 8 and 9. |                                  |           |
|    |                                                                                                                                                              |                                  |           |

TABLE 8

| Sample No. | Ink sheet No. | Image receiving sheet No. |           | Applied energy mJ/mm <sup>2</sup> |        | Power supplying period msec/line |           | Surface condition | Image unevenness | Light stability Visual | Album preservation | Number of sticking |
|------------|---------------|---------------------------|-----------|-----------------------------------|--------|----------------------------------|-----------|-------------------|------------------|------------------------|--------------------|--------------------|
|            |               | Ink                       | receiving | Applied                           | energy | power                            | supplying |                   |                  |                        |                    |                    |
| 121**      | 5             | 3                         | —         | —                                 | —      | —                                | —         | A                 | 4                | 57                     | 0.042              | 0                  |
| 122        | 5             | 3                         | 80        | 100                               | %      | 10                               | 100       | B                 | 2                | 74                     | 0.013              | 3                  |
| 123        | 5             | 3                         | 80        | 100                               |        | 9.6                              | 96        | C                 | 2                | 85                     | 0.0076             | 5                  |
| 124        | 5             | 3                         | 80        | 100                               |        | 8.6                              | 86        | C                 | 1                | 86                     | 0.0025             | 7                  |
| 125        | 5             | 3                         | 80        | 100                               |        | 7.6                              | 76        | C                 | 1                | *                      | *                  | *                  |
| 126        | 5             | 3                         | 80        | 100                               |        | 6.6                              | 66        | C                 | 1                | *                      | *                  | *                  |
| 127        | 5             | 3                         | 68        | 85                                |        | 10                               | 100       | B                 | 3                | 68                     | 0.017              | 0                  |
| 128        | 5             | 3                         | 68        | 85                                |        | 9.6                              | 96        | B                 | 3                | 79                     | 0.0115             | 0                  |
| 129        | 5             | 3                         | 68        | 85                                |        | 8.6                              | 86        | B                 | 3                | 85                     | 0.0089             | 0                  |
| 130        | 5             | 3                         | 68        | 85                                |        | 7.6                              | 76        | B                 | 3                | 87                     | 0.0064             | 0                  |
| 131        | 5             | 3                         | 68        | 85                                |        | 6.6                              | 66        | B                 | 3                | 88                     | 0.0064             | 0                  |
| 132        | 5             | 3                         | 60        | 75                                |        | 10                               | 100       | A                 | 4                | 66                     | 0.0191             | 0                  |
| 133        | 5             | 3                         | 60        | 75                                |        | 9.6                              | 96        | B                 | 4                | 76                     | 0.0127             | 0                  |
| 134        | 5             | 3                         | 60        | 75                                |        | 8.6                              | 86        | B                 | 4                | 83                     | 0.0115             | 0                  |
| 135        | 5             | 3                         | 60        | 75                                |        | 7.6                              | 76        | B                 | 4                | 86                     | 0.0089             | 0                  |
| 136        | 5             | 3                         | 60        | 75                                |        | 6.6                              | 66        | B                 | 3                | 86                     | 0.0064             | 0                  |
| 137        | 5             | 3                         | 60        | 75                                |        | 5.6                              | 56        | B                 | 3                | 86                     | 0.0064             | 0                  |
| 138        | 5             | 3                         | 50        | 63                                |        | 10                               | 100       | C                 | 4                | 64                     | 0.023              | 0                  |
| 139        | 5             | 3                         | 50        | 63                                |        | 9.6                              | 96        | C                 | 4                | 74                     | 0.0127             | 0                  |
| 140        | 5             | 3                         | 50        | 63                                |        | 8.6                              | 86        | C                 | 4                | 81                     | 0.0115             | 0                  |

\*Image receiving layer and re-heating layer are fused and evaluation was not possible.

\*\*No re-heating was applied.

TABLE 9

| Sample No. | Ink sheet No. | Image receiving sheet No. |           | Applied energy mJ/mm <sup>2</sup> |        | Power supplying period msec/line | Surface condition | Image unevenness | Light stability Visual | Album preservation | Number of sticking |   |
|------------|---------------|---------------------------|-----------|-----------------------------------|--------|----------------------------------|-------------------|------------------|------------------------|--------------------|--------------------|---|
|            |               | Ink                       | receiving | Applied                           | energy |                                  |                   |                  |                        |                    |                    |   |
| 141        | 5             | 3                         | 50        | 63                                | %      | 7.6                              | 76                | A                | 4                      | 85                 | 0.0089             | 0 |
| 142        | 5             | 3                         | 50        | 63                                |        | 6.6                              | 66                | A                | 4                      | 86                 | 0.0064             | 0 |
| 143        | 5             | 3                         | 50        | 63                                |        | 5.6                              | 56                | B                | 3                      | 86                 | 0.0064             | 0 |
| 144        | 5             | 3                         | 50        | 63                                |        | 10                               | 100               | A                | 4                      | 68                 | 0.0127             | 0 |
| 145        | 5             | 3                         | 50        | 63                                |        | 9.6                              | 96                | A                | 4                      | 79                 | 0.0064             | 0 |

TABLE 9-continued

| Sample No. | Ink sheet No. | Image receiving sheet No. | Applied energy mJ/mm <sup>2</sup> | Power supplying period msec/line | Surface condition | Image unevenness | Light stability Visual | Album preservation | Number of sticking |
|------------|---------------|---------------------------|-----------------------------------|----------------------------------|-------------------|------------------|------------------------|--------------------|--------------------|
| 146        | 5             | 3                         | 50 63                             | 8.6 86                           | A                 | 4                | 85                     | 0.0051             | 0                  |
| 147        | 5             | 3                         | 50 63                             | 7.6 76                           | A                 | 4                | 86                     | 0.0025             | 0                  |
| 148        | 5             | 3                         | 50 63                             | 6.6 66                           | A                 | 4                | 88                     | 0.0025             | 0                  |
| 149        | 5             | 3                         | 50 63                             | 5.6 56                           | B                 | 3                | 88                     | 0.0025             | 0                  |
| 150        | 5             | 3                         | 40 50                             | 10 100                           | A                 | 4                | 62                     | 0.0255             | 0                  |
| 151        | 5             | 3                         | 40 50                             | 9.6 96                           | A                 | 4                | 72                     | 0.0165             | 0                  |
| 152        | 5             | 3                         | 40 50                             | 8.6 86                           | A                 | 4                | 78                     | 0.014              | 0                  |
| 153        | 5             | 3                         | 40 50                             | 7.6 76                           | A                 | 4                | 82                     | 0.0102             | 0                  |
| 154        | 5             | 3                         | 40 50                             | 6.6 66                           | A                 | 4                | 84                     | 0.0076             | 0                  |
| 155        | 5             | 3                         | 40 50                             | 5.6 56                           | A                 | 3                | 85                     | 0.0076             | 0                  |
| 156        | 5             | 3                         | 30 38                             | 10 100                           | A                 | 4                | 59                     | 0.0293             | 0                  |
| 157        | 5             | 3                         | 30 38                             | 9.6 96                           | A                 | 4                | 70                     | 0.0178             | 0                  |
| 158        | 5             | 3                         | 30 38                             | 8.6 86                           | A                 | 4                | 75                     | 0.0127             | 0                  |
| 159        | 5             | 3                         | 30 38                             | 7.6 76                           | A                 | 4                | 79                     | 0.0102             | 0                  |
| 160        | 5             | 3                         | 30 38                             | 6.6 66                           | A                 | 4                | 82                     | 0.0089             | 0                  |

## Example 5

Yellow ink sheet, magenta ink sheet, cyan ink sheet and re-heating sheet having yellow ink layer, magenta ink layer, cyan ink layer and re-heating layer respectively were separately prepared. Composition of each layer was the same as in Example 1. Image was formed by employing the image receiving sheet 3 in the way shown in FIG. 2(c). The same result for the same evaluation was obtained as in Example 3

According to the invention, the keeping quality of a thermally transferred photographic image is improved without reducing surface characteristics, fusion of image receiving layer with ink layer, sticking of back side of ink layer with a thermal head and causing image unevenness.

What is claimed is:

1. An image forming process comprising

superposing an ink sheet on an image-receiving element, said ink sheet including an ink layer which contains a thermal transfer dye, said image-receiving element comprising an image-receiving layer adapted to accept said thermal transfer dye, whereby said ink layer is brought into contact with said image-receiving layer; imagewise treating the superposed ink sheet and the image-receiving element by a thermal head for a first time period per scanning line of said thermal head, whereby said dye of said ink sheet is transferred to the image-receiving layer to form a transferred image; bringing a thin film material into contact with an image-forming surface of said ink sheet carrying said transferred image;

reheating said transferred image by a thermal head for a second time period per scanning line of said thermal head, said second time period being shorter than said first time period; and supplying a second amount of energy to said thermal head during said reheating which is less than a first amount of energy which provides maximum density during said imagewise heating.

2. The image forming process of claim 1 wherein said second time period of said reheating is 65 to 95% of said first time period, and said second amount of energy is 40% to 80% of said first amount of energy.

3. The image forming process of claim 1 wherein the ink layer contains a thermal transfer dye precursor, and the image-receiving layer contains a dye fixing compound adapted to react with the thermal transfer dye precursor to form said thermal transfer dye.

4. The image forming process of claim 3 wherein said thermal transfer dye precursor is capable of chelation with said dye fixing compound, said dye fixing compound containing a metal ion capable of chelating with said thermal transfer dye.

5. The image forming process of claim 1 wherein said thin film material comprises a layer containing a metal ion containing compound.

6. The image forming process of claim 1 wherein the thin film material is provided as part of the ink layer.

7. The image forming process of claim 1 wherein the thin film material comprises a releasing agent.

\* \* \* \* \*